



US006187523B1

(12) **United States Patent**  
Aylward et al.

(10) **Patent No.:** US 6,187,523 B1  
(45) **Date of Patent:** Feb. 13, 2001

(54) **TOUGH IMAGING MEMBER WITH VOIDED POLYESTER SHEET**

(75) Inventors: **Peter T. Aylward**, Hilton; **Robert P. Bourdelais**, Pittsford, both of NY (US)

(73) Assignee: **Eastman Kodak Company**, Rochester, NY (US)

(\*) Notice: Under 35 U.S.C. 154(b), the term of this patent shall be extended for 0 days.

(21) Appl. No.: **09/371,658**

(22) Filed: **Aug. 10, 1999**

(51) **Int. Cl.<sup>7</sup>** ..... G03C 1/79; G03C 1/795; G03C 1/89

(52) **U.S. Cl.** ..... 430/527; 430/533; 430/534; 430/536; 430/538; 428/481; 428/483; 347/105

(58) **Field of Search** ..... 430/533, 534, 430/536, 538, 527; 347/105; 428/481, 483

(56) **References Cited**

U.S. PATENT DOCUMENTS

|           |        |                |       |           |
|-----------|--------|----------------|-------|-----------|
| 3,944,699 | 3/1976 | Mathews et al. | ..... | 428/200   |
| 4,187,113 | 2/1980 | Mathews et al. | ..... | 430/533   |
| 5,084,334 | 1/1992 | Hamano et al.  | ..... | 428/304.4 |
| 5,141,685 | 8/1992 | Maier et al.   | ..... | 264/45.3  |
| 5,143,765 | 9/1992 | Maier et al.   | ..... | 428/36.5  |

|           |   |         |                   |       |           |
|-----------|---|---------|-------------------|-------|-----------|
| 5,244,861 | * | 9/1993  | Campbell et al.   | ..... | 430/201   |
| 5,422,175 |   | 6/1995  | Ito et al.        | ..... | 428/304.4 |
| 5,431,982 |   | 7/1995  | Nishiyama et al.  | ..... | 428/141   |
| 5,866,282 |   | 2/1999  | Bourdelaïs et al. | ..... | 430/536   |
| 5,902,720 | * | 5/1999  | Haydock et al.    | ..... | 430/536   |
| 5,998,119 | * | 12/1999 | Aylward et al.    | ..... | 430/538   |
| 6,040,124 | * | 3/2000  | Aylward et al.    | ..... | 430/536   |

FOREIGN PATENT DOCUMENTS

|              |   |        |      |       |         |
|--------------|---|--------|------|-------|---------|
| 0 470 760 A2 |   | 2/1992 | (EP) | .     |         |
| 664 223 A1   | * | 7/1995 | (EP) | ..... | 430/496 |

\* cited by examiner

*Primary Examiner*—Richard L. Schilling

(74) *Attorney, Agent, or Firm*—Paul A. Leipold

(57) **ABSTRACT**

The invention relates to an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment.

**49 Claims, No Drawings**

## TOUGH IMAGING MEMBER WITH VOIDED POLYESTER SHEET

### FIELD OF THE INVENTION

This invention relates to imaging materials. In a preferred form it relates to base materials for imaging and in particular photographic reflection prints.

### BACKGROUND OF THE INVENTION

In the formation of color photographic paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper laydown and cooling of the polyethylene layers. The formation of a suitably smooth surface would also improve image quality as the photographic paper would have more apparent blackness as the reflective properties of the improved base are more spectral than the prior materials. As the whites are whiter and the blacks are blacker, there is more range in between and, therefore, contrast is enhanced.

Prior art imaging reflective papers comprise a melt extruded polyethylene layer which also serves as a carrier layer for optical brightener and other whitener materials as well as tint materials. It would be desirable if the optical brightener, whitener materials and tints, rather than being dispersed throughout the single layer of polyethylene could be concentrated nearer the surface of the layer where they would be more effective optically. The desired attributes of a quality, high impact photographic print materials are a slight blue density minimum, durability, sharpness, and flatness. Cost is also important, as print materials with a polyester substrate tend to be expensive compared with conventional material technology, mainly resin coated paper. For print materials where high levels of durability is needed, traditional color paper is undesirable, as it suffers from a lack of durability for the handling, photographic processing.

It has been proposed in U.S. Pat. No. 5,888,643 that a photographic imaging element comprising a laminated base sheet of paper with a biaxially oriented sheet within a range of Young's modulus be used to control the bending stiffness of said imaging element. While this work provides improved stiffness at a given thickness, it would be useful to provide a photographic imaging element with improved tear resistance. Having a paper base in an imaging element is desirable for its pleasing feel and its cost advantage over plastic bases. One of the disadvantages of a paper base in an imaging element is that it tends to tear easily.

In U.S. Pat. No. 5,866,282 (Bourdelaïs et al.) it is disclosed that by using microvoided biaxially oriented polyolefin sheets to a cellulose base paper where improved durability is achieved over prior art polyethylene cast coated photographic paper support materials. While this invention does provide improved durability over prior art materials there is a continuing need for tear resistant improvements to improve image durability. Further, improvements in support durability will allow more efficient web transport and stack picking in digital printing equipment such as ink jet printers.

In U.S. Pat. No. 5,866,282 (Bourdelaïs et al.) white pigments such as  $TiO_2$  are added to the biaxially oriented polyolefin sheet to provide image whiteness and sharpness. While the  $TiO_2$  added to the biaxially oriented sheet does improve whiteness and sharpness compared to melt cast

polyethylene imaging supports, there exists a processing limit to the amount of  $TiO_2$  added to polyolefin sheets. Problems such as extrusion die lines, unwanted voiding during orientation and moisture streaks. It has been found that increasing the weight percent of white pigments improves image whiteness, sharpness and opacity.

In U.S. Pat. No. 5,866,282 (Bourdelaïs et al.) biaxially oriented sheets are laminated to a base cellulose paper for use as a photographic support material. The biaxially oriented sheets described in U.S. Pat. No. 5,866,282, while tear resistant, could be improved by lowering the energy to break to allow for more efficient photographic processing. A lower energy to break would allow for the punching and chopping common to photographic processing operations to be carried out more efficiently as the cutting and punching mechanism would require less force to fracture the biaxially oriented sheets.

In U.S. Pat. No. 3,944,699 biaxially oriented polyester sheets are laminated to cellulose paper as a base for photographic prints. While the lamination of the polyester sheets does provide tear resistance, the support described in U.S. Pat. No. 3,944,699 is not suitable for a photographic print material because the paper base utilized is not sufficiently smooth, the backside film is not rough to ensure efficient web conveyance in photographic processing equipment, to obtain emulsion adhesion, expensive primer coatings are required, no compensating force exists to resist the contraction of the gelatin emulsion at relative humidity less than 50% RH and the neutral areas of the print material would appear undesirably yellow as no attempt was made to compensate for the yellowness of the gelatin commonly utilized in silver halide imaging layers.

### PROBLEM TO BE SOLVED BY THE INVENTION

There is a need for a reflective print material being more durable and having a whiter appearance.

### SUMMARY OF THE INVENTION

It is an object of the invention to overcome disadvantages of prior print materials.

It is another object to provide reflective print materials having a wider range of durability.

It is a further object to provide lower cost, high quality reflective print materials.

It is an addition object to provide an imaging element that is tear proof.

These and other objects of the invention are accomplished by an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment.

### ADVANTAGEOUS EFFECT OF THE INVENTION

The invention provides improved print materials that provide exceptional whites. The reflective print materials further provide a wider range of durability. The invention materials are more efficient in photographic processing operations.

## DETAILED DESCRIPTION OF THE INVENTION

There are numerous advantages of the invention over prior practices in the art. The invention provides a photographic element that has much less tendency to curl when exposed to extremes of humidity. Further, the invention provides a photographic paper that is may be lower in cost as the criticality's of the formation of the polyethylene are removed. There is no need for the difficult and expensive casting and cooling in forming a surface on the polyethylene layer as the biaxially oriented polymer sheet of the invention provides a high quality surface for casting of photosensitive layers. The optical properties of the photographic elements in accordance with the invention are improved as the color materials may be concentrated at the surface of the biaxially oriented sheet for most effective use with little waste of the colorant materials. Photographic materials utilizing microvoided sheets of the invention have improved resistance to tearing. The photographic materials of the invention are low in cost as the microvoided sheet may be scanned for quality prior to assembly into the photographic member. With present polyethylene layers the quality of the layer cannot be assessed until after complete formation of the base paper with the polyethylene waterproofing layer attached. Therefore, any defects result in expensive discard of expensive product. The invention allows faster hardening of photographic paper emulsion, as water vapor is not transmitted from the emulsion through the biaxially oriented sheets.

Another advantage of the microvoided polyester sheets of the invention is that they are more opaque than titanium dioxide loaded polyethylene of present products. They achieve this opacity partly by the use of the voids as well as the improved concentration of titanium dioxide at the surface of the sheet. Further, because the weight percent of  $TiO_2$  can be increased over polyolefin sheets and as a result polyester sheets tend to have better whiteness and sharpness compared to prior art biaxially oriented polyolefin sheets. The photographic elements of this invention are more scratch resistant as the oriented polyester sheet resists scratching and other damage more readily than melt cast polyethylene or oriented polyolefin sheets. These and other advantages will be apparent from the detailed description below.

In order to improve the tear resistance of an imaging support material, a biaxially oriented polyester sheet is laminated to a cellulose base paper. The biaxially oriented polyester has improve tear resistance when compared to biaxially oriented polyolefin sheets laminated to cellulose paper. Improved tear resistance has significant commercial value in that tear resistant images are perceptually preferred to images that are easily damaged. The oriented polyester sheet of this invention also has an integral emulsion adhesion layer eliminating the need for expensive subbing layers that are commonly used for polyester sheets. Levels of voiding have been optimized to provide opacity, image sharpness and whiteness without the need for white pigments.  $TiO_2$  has been added to the layers of the oriented polyester to provide improved whiteness and sharpness. The oriented polyester sheet also contains a thin color layer to offset the native yellowness of the gelatin layer typical for silver halide and ink jet receiving layers.

Unexpectedly, it has been found that oriented polyester sheets do not suffer from light exposure degradation when compared to polyolefin especially in when  $TiO_2$  is added to one or more layers. The improved stability reduces the need

for expensive light stabilizers. Further, it has been found that oriented polyester sheets have a lower surface roughness than biaxially oriented sheets improving the gloss for images formed on the support material of this invention. Because the modulus of the oriented polyester sheet is higher than the modulus of biaxially oriented polyolefin sheets, the stiffness of the imaging element can be improved.

The energy to break the oriented polyester sheets has been reduced improving the ability of the invention to fracture in chopping, punching and slitting operations common to photographic processing and roll feed digital printers compared to melt cast polyethylene or biaxially oriented polyolefin sheets.

The terms as used herein, "top", "upper", "emulsion side", and "face" mean the side or toward the side of an imaging member bearing the imaging layers. The terms "bottom", "lower side", and "back" mean the side or toward the side of the imaging member opposite from the side bearing the imaging layers or developed image. The terms used herein, "durability", "improved durability" and "tear proof" refer to improved tear resistance or tear strength of the imaging element.

Any suitable biaxially oriented polyolefin sheet may be used for the sheet on the top side of the laminated base of the invention. Microvoided composite biaxially oriented sheets are preferred and are conveniently manufactured by coextrusion of the core and surface layers, followed by biaxial orientation, whereby voids are formed around void-initiating material contained in the core layer. The layers of the coextruded polyester sheet of this invention have levels of voiding, optical brightener, and colorants adjusted to provide optimum reflection properties. The polyester sheet has a voided layer to add opacity to the base materials without the use of expensive  $TiO_2$  or other white pigments. Because the polyester base is coextruded, white pigments, optical brightener and blue tints can be concentrated in a layer just below the silver halide imaging layer significantly improving image quality and reducing the amount of white pigments, optical brightener and blue tints.

The polyester sheet of this invention preferably has a coextruded integral emulsion adhesion layer above the voided layer. The layers of the coextruded polyester sheet of this invention have levels of voiding, optical brightener, and colorants adjusted to provide optimum reflection properties.

The polyester sheet has a voided layer to add opacity to the base materials without the use of expensive  $TiO_2$  or other white pigments. Because the polyester base is coextruded, white pigments, optical brightener and blue tints can be concentrated in a layer just below the silver halide imaging layer significantly improving image quality and reducing the amount of white pigments, optical brightener and blue tints.

The polyester sheet of this invention preferably has a coextruded integral emulsion adhesion layer. Above the voided layer, a coextruded polyethylene layer can be used with corona discharge treatment as a silver halide emulsion adhesion layer, avoiding the need for a primer coating common with polyester sheets. A polyethylene layer with corona discharge treatment is preferred because gelatin based silver halide emulsions adhere well to polyethylene without the need for primer coatings. Further, the integral polyethylene skin layer preferably also contains blue tints and optical brightener to compensate for the native yellowness of the gelatin based silver halide emulsion. The voided, oriented polyester sheet of this invention is also low in cost, as the functional layer is coextruded at the same time, avoiding the need for further processing such as lamination, priming, or extrusion coating.

The polyester utilized in the invention should have a glass transition temperature between about 50° C. and about 150° C., preferably about 60–100° C., should be orientable, and have an intrinsic viscosity of at least 0.50, preferably 0.6 to 0.9. Suitable polyesters include those produced from aromatic, aliphatic, or cyclo-aliphatic dicarboxylic acids of 4–20 carbon atoms and aliphatic or alicyclic glycols having from 2–24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexane-dicarboxylic, sodiosulfoiso-phthalic, and mixtures thereof. Examples of suitable glycols include ethylene glycol, propylene glycol, butanediol, pentanediol, hexanediol, 1,4-cyclohexane-dimethanol, diethylene glycol, other polyethylene glycols and mixtures thereof. Such polyesters are well known in the art and may be produced by well-known techniques, e.g., those described in U.S. Pat. Nos. 2,465,319 and 2,901,466. Preferred continuous matrix polymers are those having repeat units from terephthalic acid or naphthalene dicarboxylic acid and at least one glycol selected from ethylene glycol, 1,4-butanediol, and 1,4-cyclohexanediethanol. Poly(ethylene terephthalate), which may be modified by small amounts of other monomers. Other suitable polyesters include liquid crystal copolymers formed by the inclusion of a suitable amount of a co-acid component such as stilbene dicarboxylic acid. Examples of such liquid crystal copolymers are those disclosed in U.S. Pat. Nos. 4,420,607; 4,459,402; and 4,468,510.

Suitable cross-linked polymers for the microbeads used in void formation during sheet formation are polymerizable organic materials which are members selected from the group consisting of an alkenyl aromatic compound having the general formula



wherein Ar represents an aromatic hydrocarbon radical, or an aromatic halohydrocarbon radical of the benzene series and R is hydrogen or the methyl radical; acrylate-type monomers including monomers of the formula



wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, and vinyl esters having the formula



wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series  $\text{HO}(\text{CH}_2)_n\text{OH}$ , wherein n is a whole number within the

range of 2–10 and having reactive olefinic linkages within the polymer molecule, the hereinabove described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, oiallyl fumarate, diallyl phthalate, and mixtures thereof.

Examples of typical monomers for making the cross-linked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, arylamidomethyl-propane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield nonuniformly sized particles, characterized by broad particle size distributions.

The resulting beads can be classified by screening to produce beads spanning the range of the original distribution of sizes. Other processes such as suspension polymerization and limited coalescence directly yield very uniformly sized particles. Suitable slip agents or lubricants include colloidal silica, colloidal alumina, and metal oxides such as tin oxide and aluminum oxide. The preferred slip agents are colloidal silica and alumina, most preferably, silica. The cross-linked polymer having a coating of slip agent may be prepared by procedures well known in the art. For example, conventional suspension polymerization processes wherein the slip agent is added to the suspension is preferred. As the slip agent, colloidal silica is preferred.

It is preferred to use the “limited coalescence” technique for producing the coated, cross-linked polymer microbeads. This process is described in detail in U.S. Pat. No. 3,615,972. Preparation of the coated microbeads for use in the present invention does not utilize a blowing agent as described in this patent, however.

The following general procedure may be utilized in a limited coalescence technique:

1. The polymerizable liquid is dispersed within an aqueous nonsolvent liquid medium to form a dispersion of droplets having sizes not larger than the size desired for the polymer globules, whereupon
2. The dispersion is allowed to rest and to reside with only mild or no agitation for a time during which a limited coalescence of the dispersed droplets takes place with the formation of a lesser number of larger droplets, such coalescence being limited due to the composition of the suspending medium, the size of the dispersed droplets thereby becoming remarkably uniform and of a desired magnitude, and
3. The uniform droplet dispersion is then stabilized by addition of thickening agents to the aqueous suspending medium, whereby the uniform-sized dispersed droplets are further protected against coalescence and are also retarded from concentrating in the dispersion due to difference in density of the disperse phase and continuous phase, and
4. The polymerizable liquid or oil phase in such stabilized dispersion is subjected to polymerization conditions and polymerized, whereby globules of polymer are obtained having spheroidal shape and remarkably uniform and desired size, which size is predetermined principally by the composition of the initial aqueous liquid suspending medium.

The diameter of the droplets of polymerizable liquid, and hence the diameter of the beads of polymer, can be varied predictably, by deliberate variation of the composition of the aqueous liquid dispersion, within the range of from about one-half of a micrometer or less to about 0.5 centimeter. For any specific operation, the range of diameters of the droplets of liquid, and hence of polymer beads, has a factor in the order of three or less as contrasted to factors of or more for diameters of droplets and beads prepared by usual suspension polymerization methods employing critical agitation procedures. Since the bead size, e.g., diameter, in the present method is determined principally by the composition of the aqueous dispersion, the mechanical conditions, such as the degree of agitation, the size and design of the apparatus used, and the scale of operation, are not highly critical. Furthermore, by employing the same composition, the operations can be repeated, or the scale of operations can be changed, and substantially the same results can be obtained.

The present method is carried out by dispersing one part by volume of a polymerizable liquid into at least 0.5, preferably from 0.5 to about 10 or more, parts by volume of a nonsolvent aqueous medium comprising water and at least the first of the following ingredients:

1. A water-dispersible, water-insoluble solid colloid, the particles of which, in aqueous dispersion, have dimensions in the order of from about 0.008 to about 50  $\mu$ m, which particles tend to gather at the liquid-liquid interface or are caused to do so by the presence of
2. A water-soluble "promotor" that affects the "hydrophilic-hydrophobic balance" of the solid colloid particles; and/or
3. An electrolyte; and/or
4. Colloid-active modifiers such as peptizing agents, surface-active agents and the like; and usually,
5. A water-soluble, monomer-insoluble inhibitor of polymerization.

The water-dispersible, water-insoluble solid colloids can be inorganic materials such as metal salts or hydroxides or clays, or can be organic materials such as raw starches, sulfonated cross-linked organic high polymers, resinous polymers, and the like.

The solid colloidal material must be insoluble but dispersible in water and both insoluble and nondispersible in, but wettable by, the polymerizable liquid. The solid colloids must be much more hydrophilic than oleophilic so as to remain dispersed wholly within the aqueous liquid. The solid colloids employed for limited coalescence are ones having particles that, in the aqueous liquid, retain a relatively rigid and discrete shape and size within the limits stated. The particles may be greatly swollen and extensively hydrated, provided that the swollen particle retains a definite shape, in which case the effective size is approximately that of the swollen particle. The particles can be essentially single molecules, as in the case of extremely high molecular weight cross-linked resins, or can be aggregates of many molecules. Materials that disperse in water to form true or colloidal solutions in which the particles have a size below the range stated or in which the particles are so diffuse as to lack a discernible shape and dimension are not suitable as stabilizers for limited coalescence. The amount of solid colloid that is employed is usually such as corresponds to from about 0.01 to about 10 or more grams per 100 cubic centimeters of the polymerizable liquid.

In order to function as a stabilizer for the limited coalescence of the polymerizable liquid droplets, it is essential that the solid colloid must tend to collect with the aqueous liquid

at the liquid-liquid interface, i.e., on the surface of the oil droplets. (The term "oil" is occasionally used herein as generic to liquids that are insoluble in water.) In many instances, it is desirable to add a "promoter" material to the aqueous composition to drive the particles of the solid colloid to the liquid-liquid interface. This phenomenon is well known in the emulsion art, and is here applied to solid colloidal particles, as an expanded of adjusting the "hydrophilic-hydrophobic balance."

Usually, the promoters are organic materials that have an affinity for the solid colloid and also for the oil droplets and that are capable of making the solid colloid more oleophilic. The affinity for the oil surface is usually due to some organic portion of the promoter molecule, while affinity for the solid colloid is usually due to opposite electrical charges. For example, positively charged complex metal salts or hydroxides, such as aluminum hydroxide, can be promoted by the presence of negatively charged organic promoters such as water-soluble sulfonated polystyrenes, alginates, and carboxymethylcellulose. Negatively charged colloids, such as Bentonite, are promoted by positively charged promoters such as tetramethyl ammonium hydroxide or chloride or water-soluble complex resinous amine condensation products, such as the water-soluble condensation products of diethanolamine and adipic acid, the water-soluble condensation products of ethylene oxide, urea and formaldehyde, and polyethylenimine. Amphoteric materials such as proteinaceous materials like gelatin, glue, casein, albumin, glutin and the like are effective promoters for a wide variety of colloidal solids. Nonionic materials like methoxy-cellulose are also effective in some instances. Usually, the promoter need be used only to the extent of a few parts per million of aqueous medium, although larger proportions can often be tolerated. In some instances, ionic materials normally classed as emulsifiers, such as soaps, long chain sulfates and sulfonates and the long chain quaternary ammonium compounds, can also be used as promoters for the solid colloids, but care must be taken to avoid causing the formation of stable colloidal emulsions of the polymerizable liquid and the aqueous liquid medium.

An effect similar to that of organic promoters is often obtained with small amounts of electrolytes, e.g., water-soluble, ionizable alkalies, acids and salts, particularly those having polyvalent ions. These are especially useful when the excessive hydrophilic or insufficient oleophilic characteristic of the colloid is attributable to excessive hydration of the colloid structure. For example, a suitably cross-linked sulfonated polymer of styrene is tremendously swollen and hydrated in water. Although the molecular structure contains benzene rings which should confer on the colloid some affinity for the oil phase in the dispersion, the great degree of hydration causes the colloidal particles to be enveloped in a cloud of associated water. The addition of a soluble, ionizable polyvalent cationic compound, such as an aluminum or calcium salt, to the aqueous composition causes extensive shrinking of the swollen colloid with exudation of a part of the associated water and exposure of the organic portion of the colloid particle, thereby making the colloid more oleophilic.

The solid colloidal particles whose hydrophilic-hydrophobic balance is such that the particles tend to gather in the aqueous phase at the oil-water interface, gather on the surface of the oil droplets and function as protective agents during limited coalescence.

Other agents that can be employed in an already known manner to effect modification of the colloidal properties of the aqueous composition are those materials known in the

art as peptizing agents, flocculating and deflocculating agents, sensitizers, surface active agents, and the like.

It is sometimes desirable to add to the aqueous liquid a few parts per million of a water-soluble, oil-insoluble inhibitor of polymerization effective to prevent the polymerization of monomer molecules that might diffuse into the aqueous liquid or that might be absorbed by colloid micelles and that, if allowed to polymerize in the aqueous phase, would tend to make emulsion-type polymer dispersions instead of, or in addition to, the desired bead or pearl polymers.

The aqueous medium containing the water-dispersible solid colloid is then admixed with the liquid polymerizable material in such a way as to disperse the liquid polymerizable material as small droplets within the aqueous medium. This dispersion can be accomplished by any usual means, e.g., by mechanical stirrers or shakers, by pumping through jets, by impingement, or by other procedures causing subdivision of the polymerizable material into droplets in a continuous aqueous medium.

The degree of dispersion, e.g., by agitation is not critical except that the size of the dispersed liquid droplets must be no larger, and is preferably much smaller, than the stable droplet size expected and desired in the stable dispersion. When such condition has been attained, the resulting dispersion is allowed to rest with only mild, gentle movement, if any, and preferably without agitation. Under such quiescent conditions, the dispersed liquid phase undergoes a limited degree of coalescence.

"Limited coalescence" is a phenomenon wherein droplets of liquid dispersed in certain aqueous suspending media coalesce, with formation of a lesser number of larger droplets, until the growing droplets reach a certain critical and limiting size, whereupon coalescence substantially ceases. The resulting droplets of dispersed liquid, which can be as large as 0.3 and sometimes 0.5 centimeter in diameter, are quite stable as regards further coalescence and are remarkably uniform in size. If such a large droplet dispersion be vigorously agitated, the droplets are fragmented into smaller droplets. The fragmented droplets, upon quiescent standing, again coalesce to the same limited degree and form the same uniform-sized, large droplet, stable dispersion. Thus, a dispersion resulting from the limited coalescence comprises droplets of substantially uniform diameter that are stable in respect to further coalescence.

The principles underlying this phenomenon have now been adapted to cause the occurrence of limited coalescence in a deliberate and predictable manner in the preparation of dispersions of polymerizable liquids in the form of droplets of uniform and desired size.

In the phenomenon of limited coalescence, the small particles of solid colloid tend to collect with the aqueous liquid at the liquid-liquid interface, i.e., on the surface of the oil droplets. It is thought that droplets which are substantially covered by such solid colloid are stable to coalescence while droplets which are not so covered are not stable. In a given dispersion of a polymerizable liquid the total surface area of the droplets is a function of the total volume of the liquid and the diameter of the droplets. Similarly, the total surface area barely coverable by the solid colloid, e.g., in a layer one particle thick, is a function of the amount of the colloid and the dimensions of the particles thereof. In the dispersion as initially prepared, e.g., by agitation, the total surface area of the polymerizable liquid droplets is greater than can be covered by the solid colloid. Under quiescent conditions, the unstable droplets begin to coalesce. The coalescence results in a decrease in the number of oil droplets and a decrease in the total surface area thereof up

to a point at which the amount of colloidal solid is barely sufficient substantially to cover the total surface of the oil droplets, whereupon coalescence substantially ceases.

If the solid colloidal particles do not have nearly identical dimensions, the average effective dimension can be estimated by statistical methods. For example, the average effective diameter of spherical particles can be computed as the square root of the average of the squares of the actual diameters of the particles in a representative sample.

It is usually beneficial to treat the uniform droplet suspension prepared as described above to render the suspension stable against congregation of the oil droplets.

This further stabilization is accomplished by gently admixing with the uniform droplet dispersion an agent capable of greatly increasing the viscosity of the aqueous liquid. For this purpose, there may be used any water-soluble or water-dispersible thickening agent that is insoluble in the oil droplets and that does not remove the layer of solid colloidal particles covering the surface of the oil droplets at the oil-water interface. Examples of suitable thickening agents are sulfonated polystyrene (water-dispersible, thickening grade), hydrophilic clays such as Bentonite, digested starch, natural gums, carboxy-substituted cellulose ethers, and the like. Often the thickening agent is selected and employed in such quantities as to form a thixotropic gel in

which are suspended the uniform-sized droplets of the oil. In other words, the thickened liquid generally should be non-Newtonian in its fluid behavior, i.e., of such a nature as to prevent rapid movement of the dispersed droplets within the aqueous liquid by the action of gravitational force due to the difference in density of the phases. The stress exerted on the surrounding medium by a suspended droplet is not sufficient to cause rapid movement of the droplet within such non-Newtonian media. Usually, the thickener agents are employed in such proportions relative to the aqueous liquid that the apparent viscosity of the thickened aqueous liquid is in the order of at least 500 centipoises (usually determined by means of a Brookfield viscosimeter using the No. 2 spindle at 30 rpm). The thickening agent is preferably prepared as a separate concentrated aqueous composition that is then carefully blended with the oil droplet dispersion.

The resulting thickened dispersion is capable of being handled, e.g., passed through pipes, and can be subjected to polymerization conditions substantially without mechanical change in the size or shape of the dispersed oil droplets.

The resulting dispersions are particularly well suited for use in continuous polymerization procedures that can be carried out in coils, tubes, and elongated vessels adapted for continuously introducing the thickened dispersions into one end and for continuously withdrawing the mass of polymer beads from the other end. The polymerization step is also practiced in batch manner.

The order of the addition of the constituents to the polymerization usually is not critical, but beneficially it is more convenient to add to a vessel the water, dispersing agent, and incorporated the oil-soluble catalyst to the monomer mixture, and subsequently add with agitation the monomer phase to the water phase.

The following is an example illustrating a procedure for preparing the cross-linked polymeric microbeads coated with slip agent. In this example, the polymer is polystyrene cross-linked with divinylbenzene. The microbeads have a coating of silica. The microbeads are prepared by a procedure in which monomer droplets containing an initiator are sized and heated to give solid polymer spheres of the same size as the monomer droplets. A water phase is prepared by combining 7 liters of distilled water, 1.5 g potassium dichro-

mate (polymerization inhibitor for the aqueous phase), 250 g polymethylaminoethanol adipate (promoter), and 350 g LUDOX (a colloidal suspension containing 50% silica sold by DuPont). A monomer phase is prepared by combining 3317 g styrene, 1421 g divinylbenzene (55% active cross-linking agent; other 45% is ethyl vinyl benzene which forms part of the styrene polymer chain) and 45 g VAZO 52 (a monomer-soluble initiator sold by DuPont). The mixture is passed through a homogenizer to obtain 5 micrometer droplets. The suspension is heated overnight at 52° C. to give 4.3 kg of generally spherical microbeads having an average diameter of about 5  $\mu\text{m}$  with narrow size distribution (about 2–10  $\mu\text{m}$  size distribution). The mol proportion of styrene and ethyl vinyl benzene to divinylbenzene is about 6.1%. The concentration of divinylbenzene can be adjusted up or down to result in about 2.5–50% (preferably 10–40%) cross-linking by the active cross-linker. Of course, monomers other than styrene and divinylbenzene can be used in similar suspension polymerization processes known in the art. Also, other initiators and promoters may be used as known in the art. Also, slip agents other than silica may also be used. For example, a number of LUDOX colloidal silicas are available from DuPont. LEPANDIN colloidal alumina is available from Degussa. NALCOAG colloidal silicas are available from Nalco, and tin oxide and titanium oxide are also available from Nalco.

Normally, for the polymer to have suitable physical properties such as resiliency, the polymer is cross-linked. In the case of styrene cross-linked with divinylbenzene, the polymer is 2.5–50% cross-linked, preferably 20–40% cross-linked. By percent cross-linked, it is meant the mol % of cross-linking agent based on the amount of primary monomer. Such limited cross-linking produces microbeads which are sufficiently coherent to remain intact during orientation of the continuous polymer. Beads of such cross-linking are also resilient, so that when they are deformed (flattened) during orientation by pressure from the matrix polymer on opposite sides of the microbeads, they subsequently resume their normal spherical shape to produce the largest possible voids around the microbeads to thereby produce articles with less density.

The microbeads are referred to herein as having a coating of a "slip agent". By this term it is meant that the friction at the surface of the microbeads is greatly reduced. Actually, it is believed this is caused by the silica acting as miniature ball bearings at the surface. Slip agent may be formed on the surface of the microbeads during their formation by including it in the suspension polymerization mix.

Microbead size is regulated by the ratio of silica to monomer. For example, the following ratios produce the indicated size microbead:

| Microbead Size, $\mu\text{m}$ | Monomer, Parts by Wt. | Slip Agent (Silica) Parts by Wt. |
|-------------------------------|-----------------------|----------------------------------|
| 2                             | 10.4                  | 1                                |
| 5                             | 27.0                  | 1                                |
| 20                            | 42.4                  | 1                                |

The microbeads of cross-linked polymer range in size from 0.1–50  $\mu\text{m}$ , and are present in an amount of 5–50% by weight based on the weight of the polyester. Microbeads of polystyrene should have a Tg of at least 20° C. higher than the Tg of the continuous matrix polymer and are hard compared to the continuous matrix polymer.

Elasticity and resiliency of the microbeads generally result in increased voiding, and it is preferred to have the Tg

of the microbeads as high above that of the matrix polymer as possible to avoid deformation during orientation. It is not believed that there is a practical advantage to cross-linking above the point of resiliency and elasticity of the microbeads.

The microbeads of cross-linked polymer are at least partially bordered by voids. The void space in the supports should occupy 2–60%, preferably 30–50%, by volume of the film support. Depending on the manner in which the supports are made, the voids may completely encircle the microbeads, e.g., a void may be in the shape of a doughnut (or flattened doughnut) encircling a micro-bead, or the voids may only partially border the microbeads, e.g., a pair of voids may border a microbead on opposite sides.

During stretching the voids assume characteristic shapes from the balanced biaxial orientation of paperlike films to the uniaxial orientation of microvoided/satinlike fibers. Balanced microvoids are largely circular in the plane of orientation, while fiber microvoids are elongated in the direction of the fiber axis. The size of the microvoids and the ultimate physical properties depend upon the degree and balance of the orientation, temperature and rate of stretching, crystallization kinetics, the size distribution of the microbeads, and the like.

The film supports according to this invention are prepared by:

- forming a mixture of molten continuous matrix polymer and cross-linked polymer wherein the cross-linked polymer is a multiplicity of microbeads uniformly dispersed throughout the matrix polymer, the matrix polymer being as described hereinbefore, the cross-linked polymer microbeads being as described hereinbefore,
- forming a film support from the mixture by extrusion or casting,
- orienting the article by stretching to form microbeads of cross-linked polymer uniformly distributed throughout the article and voids at least partially bordering the microbeads on sides thereof in the direction, or directions of orientation.

The mixture may be formed by forming a melt of the matrix polymer and mixing therein the cross-linked polymer. The cross-linked polymer may be in the form of solid or semisolid microbeads. Due to the incompatibility between the matrix polymer and cross-linked polymer, there is no attraction or adhesion between them, and they become uniformly dispersed in the matrix polymer upon mixing.

When the microbeads have become uniformly dispersed in the matrix polymer, a film support is formed by processes such as extrusion or casting. Examples of extrusion or casting would be extruding or casting a film or sheet. Such forming methods are well known in the art. If sheets or film material are cast or extruded, it is important that such article be oriented by stretching, at least in one direction. Methods of unilaterally or bilaterally orienting sheet or film material are well known in the art. Basically, such methods comprise stretching the sheet or film at least in the machine or longitudinal direction after it is cast or extruded an amount of about 1.5–10 times its original dimension. Such sheet or film may also be stretched in the transverse or cross-machine direction by apparatus and methods well known in the art, in amounts of generally 1.5–10 (usually 3–4 for polyesters and 6–10 for polypropylene) times the original dimension. Such apparatus and methods are well known in the art and are described in such U.S. Pat. No. 3,903,234.

The voids, or void spaces, referred to herein surrounding the microbeads are formed as the continuous matrix polymer

is stretched at a temperature above the Tg of the matrix polymer. The microbeads of cross-linked polymer are relatively hard compared to the continuous matrix polymer. Also, due to the incompatibility and immiscibility between the microbead and the matrix polymer, the continuous matrix polymer slides over the microbeads as it is stretched, causing voids to be formed at the sides in the direction or directions of stretch, which voids elongate as the matrix polymer continues to be stretched. Thus, the final size and shape of the voids depends on the direction(s) and amount of stretching. If stretching is only in one direction, microvoids will form at the sides of the microbeads in the direction of stretching. If stretching is in two directions (bidirectional stretching), in effect such stretching has vector components extending radially from any given position to result in a doughnut-shaped void surrounding each microbead.

The preferred preform stretching operation simultaneously opens the microvoids and orients the matrix material. The final product properties depend on and can be controlled by stretching time-temperature relationships and on the type and degree of stretch. For maximum opacity and texture, the stretching is done just above the glass transition temperature of the matrix polymer. When stretching is done in the neighborhood of the higher glass transition temperature, both phases may stretch together and opacity decreases. In the former case, the materials are pulled apart, a mechanical anticompatibilization process. Two examples are high-speed melt spinning of fibers and melt blowing of fibers and films to form nonwoven/spun-bonded products. In summary, the scope of this invention includes the complete range of forming operations just described.

In general, void formation occurs independent of, and does not require, crystalline orientation of the matrix polymer. Opaque, microvoided films have been made in accordance with the methods of this invention using completely amorphous, noncrystallizing copolymers as the matrix phase. Crystallizable/orientable (strain hardening) matrix materials are preferred for some properties like tensile strength and gas transmission barrier. On the other hand, amorphous matrix materials have special utility in other areas like tear resistance and heat sealability. The specific matrix composition can be tailored to meet many product needs. The complete range from crystalline to amorphous matrix polymer is part of the invention.

A preferred embodiment of this invention comprises an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment. Said embodiment provides a photographic element with exceptional durability and tear resistance. Said upper solid polymer layer may comprise polyethylene. Polyethylene is desirable since gelatin which is commonly used in photographic emulsion as well as ink jet receiving layer adheres to polyethylene with a simple cornea treatment as opposed to primer and subbing layer that are required polypropylene or polyesters. It is known that some copolyester and amorphous polyesters or blends with other polymer such as polyolefin may render the surface of such polymers layers slightly more compatible for adhesion with gelatin containing imaging layers. It may be feasible

when coating a multiple layers of imaging material to incorporate a sub layer of compatible latex or primer to enhance adhesion. An additional embodiment of said imaging element may incorporate tinting and or optical brighteners in said upper solid polymer. Incorporation of these material in the upper solid polymer layer is preferred because when they are concentrated in a thin layer adjacent to the image layer, there is improved efficiency and less material may be used to achieve the desired results. In the case when lower cost material such as low cost optical brightener which may be prone to migration to the surface interface between the image and the upper polymer layer are used, it may be desirable to incorporate them into a layer that is not in direct contact with the image layer.

In the process of coextrusion and subsequent biaxial orientation, when two or more layers of a polymer with different viscosities or two or more layers of different polymers are extruded simultaneous, there may be an interlayer slippage as one polymer tends to stick to the metal wall of the melt extrusion equipment and the other layer are not impeded. Such a situation may cause interlayer slippage which creates an imperfection often referred to as shark skinning. An embodiment of this invention comprises an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment and wherein at least one layer of said integrally formed biaxially oriented sheet further comprises a slip agent. There are a variety of material that may be used as a slip agent. It is further recognized that the addition of other processing aids such as metallic soaps, oligomeric fatty esters, fatty alcohol acid esters, polyolefin waxes, fatty acid esters of glycerol, dicarboxylic acid ester of fatty alcohols and even fatty acid amides may be used in combination with fluoropolymers or by themselves in lower layers of a biaxially oriented polymer sheet if the levels are kept sufficient low to minimize their interaction with the emulsion. In a preferred embodiment said slip agent comprises fluoropolymers. These polymers are preferred because they provide good compatibility with the polymers and have previously been shown to be compatible with imaging layers. The sheet of biaxially oriented polyester sheet that is adhered to both the top and bottom of a photographic paper base and said sheets contain a fluoropolymer processing aid in amount at or about 0.01 to 3% by weight. Said imaging element contains a fluoropolymer processing aid in the amount at or about 0.1 to 0.5% by weight. This range provides excellent processability during the melt extrusion and coextrusion of said sheet. In addition it has been shown that the adhesion of a photographic imaging layer is excellent over this range and the processing aid does not interfere with the wet processing of the final image or photofinishing operations.

In order to provide exceptional durability it is desirable to have said imaging element with an integrally formed biaxially oriented polymer sheet that has a modulus of at least 690 MPa. In a preferred embodiment said integrally formed biaxially oriented polymer sheet has a Young's modulus of between 690 and 15,000 MPa. A sheet with this modulus provides durability over a range of needs. Such as polymer sheet has improved tear resistance. Adhering a polyester

15

sheet to a base of paper may require that an adhesive polymer be used. In a preferred embodiment of this invention said integral layer is adhered to said base of paper utilizing a layer of melt polymer further comprising an ethylene copolymer and in particular an anhydride-modified ethylene acrylate.

The use of a voided polyester layer provides improved opacity and whiteness. The most effective use of voids in an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment wherein at least one voided layer has a void volume of between 2 and 60 percent. In this embodiment the imaging element provides added opacity without the use of  $TiO_2$  or other expense white pigment but is not fully optimize for image sharpness especially for images that are generated by optical exposure. For images that are generated by deposition of a material onto the web as in ink jet for thermal dye receiving, the amount of white pigment is not has critical for sharpness. Its role is more for developing a pleasing white appearance to the imaging element. Any white pigment known in the art may be used but  $TiO_2$  is preferred for high level of sharpness. In a preferred embodiment of said imaging element said integrally formed biaxially oriented sheet comprises titanium dioxide in an amount between 12 and 60 percent by weight. At the high end of this range, very sharp images may be achieved. An additional advantage is that as the  $TiO_2$  is concentrated, the layer comprises  $TiO_2$  may be made thinner thereby reducing the amount of polymer and pigment required. In general, thin layers with highly concentrated pigment are more efficient than thick layers. When  $TiO_2$  is used in combination with voids a synergistic benefit is achieved and the amount of  $TiO_2$  required to achieve the desired sharpness, opacity and whiteness my be lowered. This results in a more cost effective product. When  $TiO_2$  is added to a polymer and said combination is exposed to light, an oxidation process can cause the polymer to degrade and become embrittled. While polyolefins in general are more susceptible to polymer degradation than polyesters, it is may be important to protect the polymers that further comprise  $TiO_2$ . This may be especially critical when pigment is added to a voided structure since the nature of the voided layer is to have numerous cracks in the polymer layer. In another embodiment of this invention said integrally formed biaxially oriented sheet further comprises a hindered amine light stabilizer (HALS). The hindered amine will have sufficient molar mass to minimize migration in the final product, will be miscible with polyester at the preferred concentrations, and will not impart color to the final product. In the preferred embodiment, examples of HALS include poly[6-[(1,1,3,3-tetramethylbutyl)amino]-1,3,5-triazine-2,4-diyl][2,2,6,6-tetramethyl-4-piperidinyl]imino]-1,6-hexanediyil[(2,2,6,6-tetramethyl-4-piperidinyl)imino]] (such as Chimassorb 944 LD/FL), 1,3,5-triazine-2,4,6-triamine, N,N'-1,2-ethanediylbis[N-[3-[(4,6-bis[butyl(1,2,2,6,6-pentamethyl-4-piperidinyl)amino]-1,3,5-triazin-2-yl)methylamino]propyl]-N',N"-dibutyl-N',N"-bis(1,2,2,6,6-pentamethyl-4-piperidinyl)-(such as Chimassorb 119), and propanedioic acid, [[3,5-bis(1,1-dimethylethyl)-4-hydroxyphenyl]methyl]butyl-, bis(1,2,2,6,6-pentamethyl-4-piperidinyl) ester (such

16

as Tinuvin 144), although they are not limited to these compounds. In the case of said imaging element comprising a base paper having adhered to its upper surface an integrally formed biaxially oriented polymer sheet comprising at least 5 three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein 10 said upper polymer layer comprises a white pigment and wherein at least one layer may comprises polyolefin and in particular polypropylene further comprising a white pigment such as  $TiO_2$ , the layer may contain any of the hindered phenol primary antioxidants commonly used for thermal 15 stabilization of polypropylene, alone or in combination with a secondary antioxidants. Examples of hindered phenol primary antioxidants include benzenepropanoic acid, 3,5-bis(1,1-dimethylethyl)-4-hydroxy-, 2,2-bis[[3-[3-bis(1,1-dimethylethyl)-4-hydroxyphenyl]-1-oxopropoxy]methyl]-1, 3-propanediyl ester (such as Irganox 1010), benzenepropanoic acid, 3,5-bis(1,1-dimethylethyl)-4-hydroxy-, octadecyl ester (such as Irganox 1076), (such as Irganox 1035), phenol, 4,4',4"-[(2,4,6-trimethyl-1,3,5-benzenetriyl)tris(methylene)]tris[2,6-bis(1,1-dimethylethyl)-(such as Irganox 1330), but are not limited to these examples. Secondary antioxidants include organic alkyl and aryl phosphites including examples such as Phosphorous acid, bis[2,4-bis(1,1-dimethylethyl)-6-methylphenyl]ethyl ester (such as Irgafos 38), ethanamine, 2-[[2,4,8,10-tetrakis(1,1-dimethylethyl)dibenzo[d,f][1,3,2]dioxaphosphhepin-6-yl]oxy]-N,N-bis[2-[[2,4,8,10-tetrakis(1,1-dimethylethyl)dibenzo[d,f][1,3,2]dioxaphosphhepin-6-yl]oxy]ethyl] (such as Irgafos 12), phenol, 2,4-bis(1,1-dimethylethyl)-, phosphite (such as Irgafos 168). A preferred embodiment uses Irgafos 168. The combination of hindered amines with other primary and secondary antioxidants have a synergistic benefit in a multilayer biaxially oriented polymer sheet by providing thermal stability to polymers such as polypropylene during melt processing and extrusion and further enhancing their light and dark keeping properties which is not evident in a mono layer system for imaging products such as photographs. These unexpected results provide for a broader range of polymers that can be utilized 30 in imaging product, thus enabling enhanced features to be incorporated into their design.

In the area of photosensitive silver halide imaging, it is known that gelatin based emulsion are sensitive to moisture. Moisture may impact such things has the rate of hardening 50 and even the sensitometric response of the image layer. It is therefore important to control the rate of water vapor transmission. In an embodiment of this invention said integrally formed biaxially oriented sheet has a water vapor transmission rate of less than 20 g/m<sup>2</sup>/24hrs. Further, by retaining the moisture in the cellulose base paper, static charging of the support material of the invention is reduced.

When making composite imaging elements, it is often desirable to balance the structure on the bottom side of the base paper. By utilizing a biaxially oriented sheet improved 60 durability can be imparted to the element and improved curl performance. The biaxially oriented sheet may be a polyolefin sheet and in particular polypropylene which helps to bring improved cost effectiveness to the imaging element design. When additional durability is desired, the imaging element of this invention comprises at least one backside oriented sheet that comprises polyester. Such an element should have even better tear resistance. It is desirable to have

at least one backside oriented sheet that comprises a rough surface polymer layer and a layer having a modulus of greater than 690 MPa. A preferred embodiment of this invention comprises an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment and wherein said at least one backside oriented sheet is provided with indica on its upper surface. The indica may be either visible or invisible to the human eye. Indica added to an imaging element provides excellent brand identity as well as performing numerous other functions. In an additional embodiment of the imaging element of this invention said at least one backside oriented sheet is provided with a magnetic layer. The addition of a magnetic layer provides a number of opportunities to automatically encode date, time, camera and exposure information, voice recording as well as digital encoding file of the image on the other side. This would eliminate the need for expensive scanners to encode the information.

In both photographic and ink jet printing equipment there is a need to convey the imaging element through various pieces of equipment. In order to provide the proper frictional properties, the imaging element comprising a base cellulose fiber paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside oriented polymer sheet below said base paper, and wherein said upper polymer layer comprises a white pigment further comprises at least one backside oriented sheet has a bottom roughness of between 0.2 and 2.0 micrometers. This roughness provides good transportability through a variety of equipment. In another preferred embodiment said at least one backside oriented sheet is provided with a writable and conductive layer. Writability and the ability to put backmarks on the bottom side of imaging prints is desirable to help record information. Having a layer on the backside that is conductive provides a means to prevent electrostatic buildup and discharges when webs of a photographic element are being conveyed at high speed. Such discharges may cause static marks in the light sensitive layers making the print unacceptable. The use of paper as the base substrate within the imaging element of this invention further helps to minimize static by providing a base with moisture and a conductive salt to provide an internal conductive path. The use of a base paper also helps to provide an aesthetic pleasing feel to the imaging element as well as to provide an optimum stiffness to the element. This helps to assure good conveyance during photofinsihing. In an embodiment of this invention an imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer an upper solid polymer layer and below said voided polyester layer a lower solid polymer layer, and at least one backside

oriented polymer sheet below said base paper, and wherein said upper polymer layer comprises a white pigment and wherein said base paper comprises a cellulose fiber paper having a Young's modulus in the machine direction of between 2,700 and 15,000 MPa and a Young's modulus in the machine cross direction of between 1,200 and 8,000 MPa. Being able to provide a cellulose paper base with a Young's modulus as described helps to assure that the imaging element is balanced for curl in a print format as well as having good strength properties.

A preferred structure for the imaging support material of this invention where the imaging layers are applied to the polyolefin layer is as follows:

Polyethylene with red and blue tint

Polyester with 35% anatase TiO<sub>2</sub> and optical brightener

Voided polyester with a density of 0.8 g/cc

Polyester with 24% anatase TiO<sub>2</sub>

Ethylene methyl acrylate bonding layer

Cellulose paper base

Ethylene methyl acrylate bonding layer

Polyester

Copolymer of polyethylene and a terpolymer of ethylene propylene and butylene

Styrene butadiene methacrylate coating

As used herein the phrase "imaging element" is a material that may be used as a imaging support for the transfer of images to the support by techniques such as ink jet printing or thermal dye transfer as well as a support for silver halide images. As used herein, the phrase "photographic element" is a material that utilizes photosensitive silver halide in the formation of images. The thermal dye image-receiving layer of the receiving elements of the invention may comprise, for example, a polycarbonate, a polyurethane, a polyester, polyvinyl chloride, poly(styrene-co-acrylonitrile), poly(caprolactone) or mixtures thereof. The dye image-receiving layer may be present in any amount which is effective for the intended purpose. In general, good results have been obtained at a concentration of from about 1 to about 10 g/m<sup>2</sup>. An overcoat layer may be further coated over the dye-receiving layer, such as described in U.S. Pat. No. 4,775,657 of Harrison et al.

Dye-donor elements that are used with the dye-receiving element of the invention conventionally comprise a support having thereon a dye containing layer. Any dye can be used in the dye-donor employed in the invention provided it is transferable to the dye-receiving layer by the action of heat. Especially good results have been obtained with sublimable dyes. Dye donors applicable for use in the present invention are described, e.g., in U.S. Pat. Nos. 4,916,112; 4,927,803; and 5,023,228.

As noted above, dye-donor elements are used to form a dye transfer image. Such a process comprises image-wise-heating a dye-donor element and transferring a dye image to a dye-receiving element as described above to form the dye transfer image.

In a preferred embodiment of the thermal dye transfer method of printing, a dye donor element is employed which compromises a poly-(ethylene terephthalate) support coated with sequential repeating areas of cyan, magenta, and yellow dye, and the dye transfer steps are sequentially performed for each color to obtain a three-color dye transfer image. Of course, when the process is only performed for a single color, then a monochrome dye transfer image is obtained.

Thermal printing heads which can be used to transfer dye from dye-donor elements to receiving elements of the inven-

tion are available commercially. There can be employed, for example, a Fujitsu Thermal Head (FTP-040 MCS001), a TDK Thermal Head F415 HH7-1089 or a Rohm Thermal Head KE 2008-F3. Alternatively, other known sources of energy for thermal dye transfer may be used, such as lasers as described in, for example, GB No. 2,083,726A.

A thermal dye transfer assemblage of the invention comprises (a) a dye-donor element, and (b) a dye-receiving element as described above, the dye-receiving element being in a superposed relationship with the dye-donor element so that the dye layer of the donor element is in contact with the dye image-receiving layer of the receiving element.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The electrographic and electrophotographic processes and their individual steps have been well described in detail in many books and publications. The processes incorporate the basic steps of creating an electrostatic image, developing that image with charged, colored particles (toner), optionally transferring the resulting developed image to a secondary substrate, and fixing the image to the substrate. There are numerous variations in these processes and basic steps; the use of liquid toners in place of dry toners is simply one of those variations.

The first basic step, creation of an electrostatic image, can be accomplished by a variety of methods. The electrophotographic process of copiers uses imagewise photodischarge, through analog or digital exposure, of a uniformly charged photoconductor. The photoconductor may be a single-use system, or it may be rechargeable and reimagineable, like those based on selenium or organic photoreceptors.

In one form of the electrophotographic process of copiers uses imagewise photodischarge, through analog or digital exposure, of a uniformly charged photoconductor. The photoconductor may be a single-use system, or it may be rechargeable and reimagineable, like those based on selenium or organic photoreceptors.

In one form of the electrophotographic process, a photo-sensitive element is permanently imaged to form areas of differential conductivity. Uniform electrostatic charging, followed by differential discharge of the imaged element, creates an electrostatic image. These elements are called electrographic or xeroprinting masters because they can be repeatedly charged and developed after a single imaging exposure.

In an alternate electrographic process, electrostatic images are created iono-graphically. The latent image is created on dielectric (charge-holding) medium, either paper or film. Voltage is applied to selected metal styli or writing nibs from an array of styli spaced across the width of the medium, causing a dielectric breakdown of the air between the selected styli and the medium. Ions are created, which form the latent image on the medium.

Electrostatic images, however generated, are developed with oppositely charged toner particles. For development with liquid toners, the liquid developer is brought into direct contact with the electrostatic image. Usually a flowing liquid is employed, to ensure that sufficient toner particles are available for development. The field created by the electrostatic image causes the charged particles, suspended in a

nonconductive liquid, to move by electrophoresis. The charge of the latent electrostatic image is thus neutralized by the oppositely charged particles. The theory and physics of electrophoretic development with liquid toners are well described in many books and publications.

If a reimagineable photoreceptor or an electrographic master is used, the toned image is transferred to paper (or other substrate). The paper is charged electrostatically, with the polarity chosen to cause the toner particles to transfer to the paper. Finally, the toned image is fixed to the paper. For self-fixing toners, residual liquid is removed from the paper by air-drying or heating. Upon evaporation of the solvent these toners form a film bonded to the paper. For heat-fusible toners, thermoplastic polymers are used as part of the particle. Heating both removes residual liquid and fixes the toner to paper.

The dye receiving layer or DRL for ink jet imaging may be applied by any known methods. Such as solvent coating, or melt extrusion coating techniques. The DRL is coated over the TL at a thickness ranging from 0.1–10  $\mu\text{m}$ , preferably 0.5–5  $\mu\text{m}$ . There are many known formulations which may be useful as dye receiving layers. The primary requirement is that the DRL is compatible with the inks which it will be imaged so as to yield the desirable color gamut and density. As the ink drops pass through the DRL, the dyes are retained or mordanted in the DRL, while the ink solvents pass freely through the DRL and are rapidly absorbed by the TL. Additionally, the DRL formulation is preferably coated from water, exhibits adequate adhesion to the TL, and allows for easy control of the surface gloss.

For example, Misuda et al, in U.S. Pat. Nos. 4,879,166; 5,14,730; 5,264,275; 5,104,730; 4,879,166; and Japanese patents 1,095,091; 2,276,671; 2,276,670; 4,267,180; 5,024,335; and 5,016,517 discloses aqueous based DRL formulations comprising mixtures of psuedo-bohemite and certain water soluble resins. Light, in U.S. Pat. Nos. 4,903,040; 4,930,041; 5,084,338; 5,126,194; 5,126,195; 5,139,8667; and 5,147,717 discloses aqueous-based DRL formulations comprising mixtures of vinyl pyrrolidone polymers and certain water-dispersible and/or water-soluble polyesters, along with other polymers and addenda. Butters et al, in U.S. Pat. Nos. 4,857,386 and 5,102,717, disclose ink-absorbent resin layers comprising mixtures of vinyl pyrrolidone polymers and acrylic or methacrylic polymers. Sato et al., in U.S. Pat. No. 5,194,317, and Higuma et al, in U.S. Pat. No. 5,059,983, disclose aqueous-coatable DRL formulations based on poly (vinyl alcohol). Iqbal, in U.S. Pat. No. 5,208,092, discloses water-based IRL formulations comprising vinyl copolymers which are subsequently cross-linked.

In addition to these examples, there may be other known or contemplated DRL formulations which are consistent with the aforementioned primary and secondary requirements of the DRL, all of which fall under the spirit and scope of the current invention.

The preferred DRL is a 0.1–10  $\mu\text{m}$  DRL which is coated as an aqueous dispersion of 5 parts alumoxane and 5 parts poly (vinyl pyrrolidone). The DRL may also contain varying levels and sizes of matting agents for the purpose of controlling gloss, friction, and/or fingerprint resistance, surfactants to enhance surface uniformity and to adjust the surface tension of the dried coating, mordanting agents, antioxidants, UV absorbing compounds, light stabilizers, and the like.

Although the ink-receiving elements as described above can be successfully used to achieve the objectives of the present invention, it may be desirable to overcoat the DRL for the purpose of enhancing the durability of the imaged

element. Such overcoats may be applied to the DRL either before or after the element is imaged. For example, the DRL can be overcoated with an ink-permeable layer through which inks freely pass. Layers of this type are described in U.S. Pat. Nos. 4,686,118, 5,027,131, and 5,102,717. Alternatively, an overcoat may be added after the element is imaged. Any of the known laminating films and equipment may be used for this purpose. The inks used in the aforementioned imaging process are well known, and the ink formulations are often closely tied to the specific processes, i.e., continuous, piezoelectric, or thermal. Therefore, depending on the specific ink process, the inks may contain widely differing amounts and combinations of solvents, colorants, preservatives, surfactants, humectants, and the like. Inks preferred for use in combination with the image recording elements of the present invention are water-based, such as those currently sold for use in the Hewlett-Packard Desk Writer 560C printer. However, it is intended that alternative embodiments of the image-recording elements as described above, which may be formulated for use with inks which are specific to a given ink-recording process or to a given commercial vendor, fall within the scope of the present invention.

This invention is directed to a silver halide photographic element capable of excellent performance when exposed by either an electronic printing method or a conventional optical printing method. An electronic printing method comprises subjecting a radiation sensitive silver halide emulsion layer of a recording element to actinic radiation of at least  $10^{-4}$  ergs/cm<sup>2</sup> for up to  $100\mu$  seconds duration in a pixel-by-pixel mode wherein the silver halide emulsion layer is comprised of silver halide grains as described above. A conventional optical printing method comprises subjecting a radiation sensitive silver halide emulsion layer of a recording element to actinic radiation of at least  $10^{-4}$  ergs/cm<sup>2</sup> for  $10^{-3}$  to 300 seconds in an imagewise mode wherein the silver halide emulsion layer is comprised of silver halide grains as described above.

This invention in a preferred embodiment utilizes a radiation-sensitive emulsion comprised of silver halide grains (a) containing greater than 50 mole percent chloride, based on silver, (b) having greater than 50 percent of their surface area provided by {100} crystal faces, and (c) having a central portion accounting for from 95 to 99 percent of total silver and containing two dopants selected to satisfy each of the following class requirements: (i) a hexacoordination metal complex which satisfies the formula



wherein n is zero, -1, -2, -3 or -4; M is a filled frontier orbital polyvalent metal ion, other than iridium; and L<sub>6</sub> represents bridging ligands which can be independently selected, provided that least four of the ligands are anionic ligands, and at least one of the ligands is a cyano ligand or a ligand more electronegative than a cyano ligand; and (ii) an iridium coordination complex containing a thiazole or substituted thiazole ligand.

This invention is directed towards a photographic recording element comprising a support and at least one light sensitive silver halide emulsion layer comprising silver halide grains as described above.

It has been discovered quite surprisingly that the combination of dopants (i) and (ii) provides greater reduction in reciprocity law failure than can be achieved with either dopant alone. Further, unexpectedly, the combination of dopants (i) and (ii) achieve reductions in reciprocity law failure beyond the simple additive sum achieved when

employing either dopant class by itself. It has not been reported or suggested prior to this invention that the combination of dopants (i) and (ii) provides greater reduction in reciprocity law failure, particularly for high intensity and short duration exposures. The combination of dopants (i) and (ii) further unexpectedly achieves high intensity reciprocity with iridium at relatively low levels, and both high and low intensity reciprocity improvements even while using conventional gelatino-peptizer (e.g., other than low methionine gelatino-peptizer).

In a preferred practical application, the advantages of the invention can be transformed into increased throughput of digital substantially artifact-free color print images while exposing each pixel sequentially in synchronism with the digital data from an image processor.

In one embodiment, the present invention represents an improvement on the electronic printing method. Specifically, this invention in one embodiment is directed to an electronic printing method which comprises subjecting a radiation sensitive silver halide emulsion layer of a recording element to actinic radiation of at least  $10^{-4}$  ergs/cm<sup>2</sup> for up to  $100\mu$  seconds duration in a pixel-by-pixel mode. The present invention realizes an improvement in reciprocity failure by selection of the radiation sensitive silver halide emulsion layer. While certain embodiments of the invention are specifically directed towards electronic printing, use of the emulsions and elements of the invention is not limited to such specific embodiment, and it is specifically contemplated that the emulsions and elements of the invention are also well suited for conventional optical printing.

It has been unexpectedly discovered that significantly improved reciprocity performance can be obtained for silver halide grains (a) containing greater than 50 mole percent chloride, based on silver, and (b) having greater than 50 percent of their surface area provided by {100} crystal faces by employing a hexacoordination complex dopant of class (i) in combination with an iridium complex dopant comprising a thiazole or substituted thiazole ligand. The reciprocity improvement is obtained for silver halide grains employing conventional gelatino-peptizer, unlike the contrast improvement described for the combination of dopants set forth in U.S. Pat. Nos. 5,783,373 and 5,783,378, which requires the use of low methionine gelatino-peptizers as discussed therein, and which states it is preferable to limit the concentration of any gelatino-peptizer with a methionine level of greater than 30 micromoles per gram to a concentration of less than 1 percent of the total peptizer employed. Accordingly, in specific embodiments of the invention, it is specifically contemplated to use significant levels (i.e., greater than 1 weight percent of total peptizer) of conventional gelatin (e.g., gelatin having at least 30 micromoles of methionine per gram) as a gelatino-peptizer for the silver halide grains of the emulsions of the invention. In preferred embodiments of the invention, gelatino-peptizer is employed which comprises at least 50 weight percent of gelatin containing at least 30 micromoles of methionine per gram, as it is frequently desirable to limit the level of oxidized low methionine gelatin which may be used for cost and certain performance reasons.

In a specific, preferred form of the invention it is contemplated to employ a class (i) hexacoordination complex dopant satisfying the formula:



where

n is zero, -1, -2, -3 or -4;  
M is a filled frontier orbital polyvalent metal ion, other than iridium, preferably  $Fe^{+2}$ ,  $Ru^{+2}$ ,  $Os^{+2}$ ,  $Co^{+3}$ ,  $Rh^{+3}$ ,

Pd<sup>+4</sup> or Pt<sup>+4</sup>, more preferably an iron, ruthenium or osmium ion, and most preferably a ruthenium ion; L<sub>6</sub> represents six bridging ligands which can be independently selected, provided that at least four of the ligands are anionic ligands and at least one (preferably at least 3 and optimally at least 4) of the ligands is a cyano ligand or a ligand more electronegative than a cyano ligand. Any remaining ligands can be selected from among various other bridging ligands, including aquo ligands, halide ligands (specifically, fluoride, chloride, bromide and iodide), cyanate ligands, thiocyanate ligands, selenocyanate ligands, tellurocyanate ligands, and azide ligands. Hexacoordinated transition metal complexes of class (i) which include six cyano ligands are specifically preferred.

Illustrations of specifically contemplated class (i) hexacoordination complexes for inclusion in the high chloride grains are provided by Olm et al U.S. Pat. No. 5,503,970 and Daubendiek et al U.S. Pat. Nos. 5,494,789 and 5,503,971, and Keevert et al U.S. Pat. No. 4,945,035, as well as Murakami et al Japanese Patent Application Hei-2[1990]-249588, and Research Disclosure Item 36736. Useful neutral and anionic organic ligands for class (ii) dopant hexacoordination complexes are disclosed by Olm et al U.S. Pat. No. 5,360,712 and Kuromoto et al U.S. Pat. No. 5,462,849.

Class (i) dopant is preferably introduced into the high chloride grains after at least 50 (most preferably 75 and optimally 80) percent of the silver has been precipitated, but before precipitation of the central portion of the grains has been completed. Preferably class (i) dopant is introduced before 98 (most preferably 95 and optimally 90) percent of the silver has been precipitated. Stated in terms of the fully precipitated grain structure, class (i) dopant is preferably present in an interior shell region that surrounds at least 50 (most preferably 75 and optimally 80) percent of the silver and, with the more centrally located silver, accounts for the entire central portion (99 percent of the silver), most preferably accounts for 95 percent, and optimally accounts for 90 percent of the silver halide forming the high chloride grains. The class (i) dopant can be distributed throughout the interior shell region delimited above or can be added as one or more bands within the interior shell region.

Class (i) dopant can be employed in any conventional useful concentration. A preferred concentration range is from 10<sup>-8</sup> to 10<sup>-3</sup> mole per silver mole, most preferably from 10<sup>-6</sup> to 5×10<sup>-4</sup> mole per silver mole.

The following are specific illustrations of class (i) dopants:

- (i-1) [Fe(CN)<sub>6</sub>]<sup>-4</sup>
- (i-2) [Ru(CN)<sub>6</sub>]<sup>-4</sup>
- (i-3) [Os(CN)<sub>6</sub>]<sup>-4</sup>
- (i-4) [Rh(CN)<sub>6</sub>]<sup>-3</sup>
- (i-5) [Co(CN)<sub>6</sub>]<sup>-3</sup>
- (i-6) [Fe(pyrazine)(CN)<sub>5</sub>]<sup>-4</sup>
- (i-7) [RuCl(CN)<sub>5</sub>]<sup>-4</sup>
- (i-8) [OsBr(CN)<sub>5</sub>]<sup>-4</sup>
- (i-9) [RhF(CN)<sub>5</sub>]<sup>-3</sup>
- (i-10) [In(NCS)<sub>6</sub>]<sup>-3</sup>
- (i-11) [FeCO(CN)<sub>5</sub>]<sup>-3</sup>
- (i-12) [RuF<sub>2</sub>(CN)<sub>4</sub>]<sup>-4</sup>
- (i-13) [OsCl<sub>2</sub>(CN)<sub>4</sub>]<sup>-4</sup>
- (i-14) [RhL<sub>2</sub>(CN)<sub>4</sub>]<sup>-3</sup>
- (i-15) [Ga(NCS)<sub>6</sub>]<sup>-3</sup>
- (i-16) [Ru(CN)<sub>5</sub>(OCN)]<sup>-4</sup>
- (i-17) [Ru(CN)<sub>5</sub>(N<sub>3</sub>)]<sup>-4</sup>
- (i-18) [Os(CN)<sub>5</sub>(SCN)]<sup>-4</sup>
- (i-19) [Rh(CN)<sub>5</sub>(SeCN)]<sup>-3</sup>

(i-20) [Os(CN)Cl<sub>5</sub>]<sup>-4</sup>  
(i-21) [Fe(CN)<sub>3</sub>Cl<sub>3</sub>]<sup>-3</sup>  
(i-22) [Ru(CO)<sub>2</sub>(CN)<sub>4</sub>]<sup>-1</sup>

When the class (i) dopants have a net negative charge, it is appreciated that they are associated with a counter ion when added to the reaction vessel during precipitation. The counter ion is of little importance, since it is ionically dissociated from the dopant in solution and is not incorporated within the grain. Common counter ions known to be fully compatible with silver chloride precipitation, such as ammonium and alkali metal ions, are contemplated. It is noted that the same comments apply to class (ii) dopants, otherwise described below.

The class (ii) dopant is an iridium coordination complex containing at least one thiazole or substituted thiazole ligand. Careful scientific investigations have revealed Group VIII hexahalo coordination complexes to create deep electron traps, as illustrated R. S. Eachus, R. E. Graves and M. T. Olm *J. Chem. Phys.*, Vol. 69, pp. 4580-7 (1978) and *Physica Status Solidi A*, Vol. 57, 429-37 (1980) and R. S. Eachus and M. T. Olm *Annu. Rep. Prog. Chem. Sect. C. Phys. Chem.*, Vol. 83, 3, pp. 3-48 (1986). The class (ii) dopants employed in the practice of this invention are believed to create such deep electron traps. The thiazole ligands may be substituted with any photographically acceptable substituent which does not prevent incorporation of the dopant into the silver halide grain. Exemplary substituents include lower alkyl (e.g., alkyl groups containing 1-4 carbon atoms), and specifically methyl. A specific example of a substituted thiazole ligand which may be used in accordance with the invention is 5-methylthiazole. The class (ii) dopant preferably is an iridium coordination complex having ligands each of which are more electropositive than a cyano ligand. In a specifically preferred form the remaining non-thiazole or nonsubstituted-thiazole ligands of the coordination complexes forming class (ii) dopants are halide ligands.

It is specifically contemplated to select class (ii) dopants from among the coordination complexes containing organic ligands disclosed by Olm et al U.S. Pat. No. 5,360,712, Olm et al U.S. Pat. No. 5,457,021 and Kuromoto et al U.S. Pat. No. 5,462,849.

In a preferred form it is contemplated to employ as a class (ii) dopant a hexacoordination complex satisfying the formula:



wherein

50 n' is zero, -1, -2, -3 or -4; and L<sup>1</sup><sub>6</sub> represents six bridging ligands which can be independently selected, provided that at least four of the ligands are anionic ligands, each of the ligands is more electropositive than a cyano ligand, and at least one of the ligands comprises a thiazole or substituted thiazole ligand. In a specifically preferred form at least four of the ligands are halide ligands, such as chloride or bromide ligands.

Class (ii) dopant is preferably introduced into the high chloride grains after at least 50 (most preferably 85 and optimally 90) percent of the silver has been precipitated, but before precipitation of the central portion of the grains has been completed. Preferably class (ii) dopant is introduced before 99 (most preferably 97 and optimally 95) percent of the silver has been precipitated. Stated in terms of the fully precipitated grain structure, class (ii) dopant is preferably present in an interior shell region that surrounds at least 50

(most preferably 85 and optimally 90) percent of the silver and, with the more centrally located silver, accounts the entire central portion (99 percent of the silver), most preferably accounts for 97 percent, and optimally accounts for 95 percent of the silver halide forming the high chloride grains. The class (ii) dopant can be distributed throughout the interior shell region delimited above or can be added as one or more bands within the interior shell region.

Class (ii) dopant can be employed in any conventional useful concentration. A preferred concentration range is from  $10^{-9}$  to  $10^{-4}$  mole per silver mole. Iridium is most preferably employed in a concentration range of from  $10^{-8}$  to  $10^{-5}$  mole per silver mole.

Specific illustrations of class (ii) dopants are the following:

- (ii-1)  $[\text{IrCl}_5(\text{thiazole})]^{-2}$
- (ii-2)  $[\text{IrCl}_4(\text{thiazole})_2]^{-1}$
- (ii-3)  $[\text{IrBr}_5(\text{thiazole})]^{-2}$
- (ii-4)  $[\text{IrBr}_4(\text{thiazole})_2]^{-1}$
- (ii-5)  $[\text{IrCl}_5(5\text{-methylthiazole})]^{-2}$
- (ii-6)  $[\text{IrCl}_4(5\text{-methylthiazole})_2]^{-1}$
- (ii-7)  $[\text{IrBr}_5(5\text{-methylthiazole})]^{-2}$
- (ii-8)  $[\text{IrBr}_4(5\text{-methylthiazole})_2]^{-1}$

In one preferred aspect of the invention in a layer using a magenta dye forming coupler, a class (ii) dopant in combination with an  $\text{OsCl}_5(\text{NO})$  dopant has been found to produce a preferred result.

Emulsions demonstrating the advantages of the invention can be realized by modifying the precipitation of conventional high chloride silver halide grains having predominantly (>50%) {100} crystal faces by employing a combination of class (i) and (ii) dopants as described above.

The silver halide grains precipitated contain greater than 50 mole percent chloride, based on silver. Preferably the grains contain at least 70 mole percent chloride and, optimally at least 90 mole percent chloride, based on silver. Iodide can be present in the grains up to its solubility limit, which is in silver iodochloride grains, under typical conditions of precipitation, about 11 mole percent, based on silver. It is preferred for most photographic applications to limit iodide to less than 5 mole percent iodide, most preferably less than 2 mole percent iodide, based on silver.

Silver bromide and silver chloride are miscible in all proportions. Hence, any portion, up to 50 mole percent, of the total halide not accounted for chloride and iodide, can be bromide. For color reflection print (i.e., color paper) uses bromide is typically limited to less than 10 mole percent based on silver and iodide is limited to less than 1 mole percent based on silver.

In a widely used form high chloride grains are precipitated to form cubic grains—that is, grains having {100} major faces and edges of equal length. In practice ripening effects usually round the edges and comers of the grains to some extent. However, except under extreme ripening conditions substantially more than 50 percent of total grain surface area is accounted for by {100} crystal faces.

High chloride tetradechedral grains are a common variant of cubic grains. These grains contain 6 {100} crystal faces and 8 {111} crystal faces. Tetradechedral grains are within the contemplation of this invention to the extent that greater than 50 percent of total surface area is accounted for by {100} crystal faces.

Although it is common practice to avoid or minimize the incorporation of iodide into high chloride grains employed in color paper, it is has been recently observed that silver iodochloride grains with {100} crystal faces and, in some instances, one or more {111} faces offer exceptional levels

of photographic speed. In the these emulsions iodide is incorporated in overall concentrations of from 0.05 to 3.0 mole percent, based on silver, with the grains having a surface shell of greater than 50 Å thickness that is substantially free of iodide and a interior shell having a maximum iodide concentration that surrounds a core accounting for at least 50 percent of total silver. Such grain structures are illustrated by Chen et al EPO 0 718 679.

In another improved form the high chloride grains can take the form of tabular grains having {100} major faces. Preferred high chloride {100} tabular grain emulsions are those in which the tabular grains account for at least 70 (most preferably at least 90) percent of total grain projected area. Preferred high chloride {100} tabular grain emulsions

have average aspect ratios of at least (most preferably at least >8). Tabular grains typically have thicknesses of less than 0.3  $\mu\text{m}$ , preferably less than 0.2  $\mu\text{m}$ , and optimally less than 0.07  $\mu\text{m}$ . High chloride {100} tabular grain emulsions and their preparation are disclosed by Maskasky U.S. Pat. Nos. 5,264,337 and 5,292,632, House et al U.S. Pat. No. 5,320,938, Brust et al U.S. Pat. No. 5,314,798 and Chang et al U.S. Pat. No. 5,413,904.

Once high chloride grains having predominantly {100} crystal faces have been precipitated with a combination of class (i) and class (ii) dopants described above, chemical and spectral sensitization, followed by the addition of conventional addenda to adapt the emulsion for the imaging application of choice can take any convenient conventional form. These conventional features are illustrated by Research Disclosure, Item 38957, cited above, particularly:

- III. Emulsion washing;
- IV. Chemical sensitization;
- V. Spectral sensitization and desensitization;
- VII. Antifoggants and stabilizers;
- VIII. Absorbing and scattering materials;
- IX. Coating and physical property modifying addenda; and
- X. Dye image formers and modifiers.

Some additional silver halide, typically less than 1 percent, based on total silver, can be introduced to facilitate chemical sensitization. It is also recognized that silver halide can be epitaxially deposited at selected sites on a host grain to increase its sensitivity. For example, high chloride {100} tabular grains with corner epitaxy are illustrated by Maskasky U.S. Pat. No. 5,275,930. For the purpose of providing a clear demarcation, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains while silver halide that deposits and provides the final {100} crystal faces of the grains is included in the total silver forming the grains, even when it differs significantly in composition from the previously precipitated silver halide.

In the simplest contemplated form a recording element contemplated for use in the electronic printing method of one embodiment of the invention can consist of a single emulsion layer satisfying the emulsion description provided above coated on a conventional photographic support, such as those described in Research Disclosure, Item 38957, cited above, XVI. Supports. In one preferred form the support is a white reflective support, such as photographic paper sup-

port or a film support that contains or bears a coating of a reflective pigment. To permit a print image to be viewed using an illuminant placed behind the support, it is preferred to employ a white translucent support, such as a Duratrans™ or Duraclear™ support.

Image dye-forming couplers may be included in the element such as couplers that form cyan dyes upon reaction with oxidized color developing agents which are described in such representative patents and publications as: U.S. Pat. Nos. 2,367,531; 2,423,730; 2,474,293; 2,772,162; 2,895,826; 3,002,836; 3,034,892; 3,041,236; 4,883,746 and "Farbkuppler-Eine Literature Ubersicht," published in Agfa Mitteilungen, Band III, pp. 156-175 (1961). Preferably such couplers are phenols and naphthols that form cyan dyes on reaction with oxidized color developing agent. Also preferable are the cyan couplers described in, for instance, European Patent Application Nos. 491,197; 544,322; 556,700; 556,777; 565,096; 570,006; and 574,948.

Typical cyan couplers are represented by the following formulas:



wherein R<sub>1</sub>, R<sub>5</sub> and R<sub>8</sub> each represent a hydrogen or a substituent; R<sub>2</sub> represents a substituent; R<sub>3</sub>, R<sub>4</sub> and R<sub>7</sub> each represent an electron attractive group having a Hammett's substituent constant  $\sigma_{para}$  of 0.2 or more and the sum of the  $\sigma_{para}$  values of R<sub>3</sub> and R<sub>4</sub> is 0.65 or more; R<sub>6</sub> represents an electron attractive group having a Hammett's substituent constant  $\sigma_{para}$  of 0.35 or more; X represents a hydrogen or a coupling-off group; Z<sub>1</sub> represents nonmetallic atoms necessary for forming a nitrogen-containing, six-membered, heterocyclic ring which has at least one dissociative group; Z<sub>2</sub> represents  $-C(R_7)=$  and  $-N=$ ; and Z<sub>3</sub> and Z<sub>4</sub> each represent  $-C(R_8)=$  and  $-N=$ .

For purposes of this invention, an "NB coupler" is a dye-forming coupler which is capable of coupling with the developer 4-amino-3-methylthiyl-N-ethyl-N-(2-methanesulfonamidoethyl) aniline sesquisulfate hydrate to form a dye for which the left bandwidth (LBW) of its absorption spectra upon "spin coating" of a 3% w/v solution

of the dye in di-n-butyl sebacate solvent is at least 5 nm. less than the LBW for a 3% w/v solution of the same dye in acetonitrile. The LBW of the spectral curve for a dye is the distance between the left side of the spectral curve and the wavelength of maximum absorption measured at a density of half the maximum.

The "spin coating" sample is prepared by first preparing a solution of the dye in di-n-butyl sebacate solvent (3% w/v). If the dye is insoluble, dissolution is achieved by the addition of some methylene chloride. The solution is filtered and 0.1-0.2 ml is applied to a clear polyethylene terephthalate support (approximately 4 cm×4 cm) and spun at 4,000 RPM using the Spin Coating equipment, Model No. EC101, available from Headway Research Inc., Garland Tex. The transmission spectra of the so prepared dye samples are then recorded.

Preferred "NB couplers" form a dye which, in n-butyl sebacate, has a LBW of the absorption spectra upon "spin coating" which is at least 15 nm, preferably at least 25 nm, less than that of the same dye in a 3% solution (w/v) in acetonitrile.

In a preferred embodiment the cyan dye-forming "NB coupler" useful in the invention has the formula (IA)



30 CYAN-3 35 wherein

R' and R'' are substituents selected such that the coupler is a "NB coupler", as herein defined; and

Z is a hydrogen atom or a group which can be split off by the reaction of the coupler with an oxidized color developing agent.

The coupler of formula (IA) is a 2,5-diamido phenolic cyan coupler wherein the substituents R' and R'' are preferably independently selected from unsubstituted or substituted alkyl, aryl, amino, alkoxy and heterocycl groups.

40 45 In a further preferred embodiment, the "NB coupler" has the formula (I):



wherein

R' and R'' are independently selected from unsubstituted or substituted alkyl, aryl, amino, alkoxy and heterocycl groups and Z is as hereinbefore defined;

R<sub>1</sub> and R<sub>2</sub> are independently hydrogen or an unsubstituted or substituted alkyl group; and

Typically, R'' is an alkyl, amino or aryl group, suitably a phenyl group. R''' is desirably an alkyl or aryl group or a

5-10 membered heterocyclic ring which contains one or more heteroatoms selected from nitrogen, oxygen and sulfur, which ring group is unsubstituted or substituted.

In the preferred embodiment the coupler of formula (I) is a 2,5-diamido phenol in which the 5-amido moiety is an amide of a carboxylic acid which is substituted in the alpha position by a particular sulfone ( $-\text{SO}_2-$ ) group, such as, for example, described in U.S. Pat. No. 5,686,235. The sulfone moiety is an unsubstituted or substituted alkylsulfone or a heterocyclyl sulfone or it is an arylsulfone, which is preferably substituted, in particular in the meta and/or para position.

Couplers having these structures of formulae (I) or (IA) comprise cyan dye-forming "NB couplers" which form image dyes having very sharp-cutting dye hues on the short wavelength side of the absorption curves with absorption maxima ( $\lambda_{max}$ ) which are shifted hypsochromically and are generally in the range of 620-645 nm, which is ideally suited for producing excellent color reproduction and high color saturation in color photographic papers.

Referring to formula (I),  $R_1$  and  $R_2$  are independently hydrogen or an unsubstituted or substituted alkyl group, preferably having from 1 to 24 carbon atoms and in particular 1 to 10 carbon atoms, suitably a methyl, ethyl, n-propyl, isopropyl, butyl or decyl group or an alkyl group substituted with one or more fluoro, chloro or bromo atoms, such as a trifluoromethyl group. Suitably, at least one of  $R_1$  and  $R_2$  is a hydrogen atom and if only one of  $R_1$  and  $R_2$  is a hydrogen atom then the other is preferably an alkyl group having 1 to 4 carbon atoms, more preferably one to three carbon atoms and desirably two carbon atoms.

As used herein and throughout the specification unless where specifically stated otherwise, the term "alkyl" refers to an unsaturated or saturated straight or branched chain alkyl group, including alkenyl, and includes aralkyl and cyclic alkyl groups, including cycloalkenyl, having 3-8 carbon atoms and the term 'aryl' includes specifically fused aryl.

In formula (I),  $R''$  is suitably an unsubstituted or substituted amino, alkyl or aryl group or a 5-10 membered heterocyclic ring which contains one or more heteroatoms selected from nitrogen, oxygen and sulfur, which ring is unsubstituted or substituted, but is more suitably an unsubstituted or substituted phenyl group.

Examples of suitable substituent groups for this aryl or heterocyclic ring include cyano, chloro, fluoro, bromo, iodo, alkyl- or aryl-carbonyl, alkyl- or aryl-oxy carbonyl, carbonamido, alkyl- or aryl-carbonamido, alkyl- or aryl-sulfonyl, alkyl- or aryl-sulfonyloxy, alkyl- or aryl-oxysulfonyl, alkyl- or aryl-sulfoxide, alkyl- or aryl-sulfamoyl, alkyl- or aryl-sulfonamido, aryl, alkyl, alkoxy, aryloxy, nitro, alkyl- or aryl-ureido and alkyl- or aryl-carbamoyl groups, any of which may be further substituted. Preferred groups are halogen, cyano, alkoxy carbonyl, alkylsulfamoyl, alkyl-sulfonamido, alkylsulfonyl, carbamoyl, alkylcarbamoyl or alkylcarbonamido. Suitably,  $R''$  is a 4-chlorophenyl, 3,4-dichlorophenyl, 3,4-difluorophenyl, 4-cyanophenyl, 3-chloro-4-cyanophenyl, pentafluorophenyl, or a 3- or 4-sulfonamidophenyl group.

In formula (I), when  $R''$  is alkyl it may be unsubstituted or substituted with a substituent such as halogen or alkoxy. When  $R''$  is aryl or a heterocycle, it may be substituted. Desirably it is not substituted in the position alpha to the sulfonyl group.

In formula (I), when  $R''$  is a phenyl group, it may be substituted in the meta and/or para positions with one to three substituents independently selected from the group

consisting of halogen, and unsubstituted or substituted alkyl, alkoxy, aryloxy, acyloxy, acylamino, alkyl- or arylsulfonyloxy, alkyl- or aryl-sulfamoyl, alkyl- or arylsulfamoylamino, alkyl- or aryl-sulfonamido, alkyl- or arylureido, alkyl- or aryl-oxy carbonyl, alkyl- or aryl-oxy carbonylamino and alkyl- or aryl-carbamoyl groups.

In particular each substituent may be an alkyl group such as methyl, t-butyl, heptyl, dodecyl, pentadecyl, octadecyl or 1,1,2,2-tetramethylpropyl; an alkoxy group such as methoxy, t-butoxy, octyloxy, dodecyloxy, tetradecyloxy, hexadecyloxy or octadecyloxy; an aryloxy group such as phenoxy, 4-t-butylphenoxy or 4-dodecyl-phenoxy; an alkyl- or aryl-acyloxy group such as acetoxy or dodecanoyloxy; an alkyl- or aryl-acylamino group such as acetamido, hexadecanamido or benzamido; an alkyl- or aryl-sulfonyloxy group such as methyl-sulfonyloxy, dodecylsulfonyloxy or 4-methylphenyl-sulfonyloxy; an alkyl- or aryl-sulfamoyl group such as N-butylsulfamoyl or N-4-t-butylphenylsulfamoyl; an alkyl- or aryl-sulfamoylamino group such as N-butylsulfamoylamino or N-4-t-butylphenylsulfamoyl-amino; an alkyl- or aryl-sulfonamido group such as methane-sulfonamido, hexadecanesulfonamido or 4-chlorophenyl-sulfonamido; an alkyl- or arylureido group such as methylureido or phenylureido; an alkoxy- or aryloxy-carbonyl such as methoxycarbonyl or phenoxy carbonyl; an alkoxy- or aryloxy-carbonylamino group such as methoxy-carbonylamino or phenoxy carbonylamino; an alkyl- or aryl-carbamoyl group such as N-butylcarbamoyl or N-methyl-N-dodecylcarbamoyl; or a perfluoroalkyl group such as trifluoromethyl or heptafluoropropyl.

Suitably the above substituent groups have 1 to 30 carbon atoms, more preferably 8 to 20 aliphatic carbon atoms. A desirable substituent is an alkyl group of 12 to 18 aliphatic carbon atoms such as dodecyl, pentadecyl or octadecyl or an alkoxy group with 8 to 18 aliphatic carbon atoms such as dodecyloxy and hexadecyloxy or a halogen such as a meta or para chloro group, carboxy or sulfonamido. Any such groups may contain interrupting heteroatoms such as oxygen to form e.g. polyalkylene oxides.

In formula (I) or (IA)  $Z$  is a hydrogen atom or a group which can be split off by the reaction of the coupler with an oxidized color developing agent, known in the photographic art as a 'coupling-off group' and may preferably be hydrogen, chloro, fluoro, substituted aryloxy or mercaptotetrazole, more preferably hydrogen or chloro.

The presence or absence of such groups determines the chemical equivalency of the coupler, i.e., whether it is a 2-equivalent or 4-equivalent coupler, and its particular identity can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction, and the like.

Representative classes of such coupling-off groups include, for example, halogen, alkoxy, aryloxy, heterocyclloxy, sulfonyloxy, acyloxy, acyl, heterocyclsulfonamido, heterocyclthio, benzothiazolyl, phosphonyloxy, alkylthio, arylthio, and arylazo. These coupling-off groups are described in the art, for example, in U.S. Pat. Nos. 2,455,169, 3,227,551, 3,432,521, 3,467,563, 3,617,291, 3,880,661, 4,052,212, and 4,134,766; and in U.K. Patent Nos. and published applications 1,466,728, 1,531,927, 1,533,039, 2,066,755A, and 2,017,704A, the

31

disclosures of which are incorporated herein by reference. Halogen, alkoxy and aryloxy groups are most suitable.

Examples of specific coupling-off groups are  $-\text{Cl}$ ,  $-\text{F}$ ,  $-\text{Br}$ ,  $-\text{SCN}$ ,  $-\text{OCH}_3$ ,  $-\text{OC}_6\text{H}_5$ ,  $-\text{OCH}_2\text{C}(=\text{O})$   $\text{NHCH}_2\text{CH}_2\text{OH}$ ,  $-\text{OCH}_2\text{C}(\text{O})\text{NHCH}_2\text{CH}_2\text{OCH}_3$ ,  $-\text{OCH}_2\text{C}(\text{O})\text{NHCH}_2\text{CH}_2\text{OC}(=\text{O})\text{OCH}_3$ ,  $-\text{P}(=\text{O})(\text{OC}_2\text{H}_5)_2$ ,  $-\text{SCH}_2\text{CH}_2\text{COOH}$ ,



Typically, the coupling-off group is a chlorine atom, hydrogen atom or p-methoxyphenoxy group.

It is essential that the substituent groups be selected so as to adequately ballast the coupler and the resulting dye in the organic solvent in which the coupler is dispersed. The ballasting may be accomplished by providing hydrophobic substituent groups in one or more of the substituent groups. Generally a ballast group is an organic radical of such size and configuration as to confer on the coupler molecule sufficient bulk and aqueous insolubility as to render the coupler substantially nondiffusible from the layer in which it is coated in a photographic element. Thus the combination of substituent are suitably chosen to meet these criteria. To be effective, the ballast will usually contain at least 8 carbon atoms and typically contains 10 to 30 carbon atoms. Suitable ballasting may also be accomplished by providing a plurality of groups which in combination meet these criteria. In the preferred embodiments of the invention  $R_1$  in formula (I) is a small alkyl group or hydrogen. Therefore, in these embodiments the ballast would be primarily located as part of the

32

other groups. Furthermore, even if the coupling-off group Z contains a ballast it is often necessary to ballast the other substituents as well, since Z is eliminated from the molecule upon coupling; thus, the ballast is most advantageously provided as part of groups other than Z.

The following examples further illustrate preferred coupler of the invention. It is not to be construed that the present invention is limited to these examples.



**33**

-continued

**34**

-continued

IC-9



**35**

-continued



IC-13



IC-17



IC-14



IC-18



IC-15



IC-19



IC-16



IC-20

**37**

-continued

**38**

-continued

IC-25



IC-27



IC-28



**39**

-continued



IC-29

**40**

-continued



IC-33

IC-30



20



IC-34

IC-31



35



IC-35

IC-32



55



IC-36

41

-continued



42

Preferred couplers are IC-3, IC-7, IC-35, and IC-36 because of their suitably narrow left bandwidths.

Couplers that form magenta dyes upon reaction with oxidized color developing agent are described in such representative patents and publications as: U.S. Pat. Nos. 2,311,082; 2,343,703; 2,369,489; 2,600,788; 2,908,573; 3,062,653; 3,152,896; 3,519,429; 3,758,309; and "Farbkuppler-eine Literature Ubersicht," published in Agfa Mitteilungen, Band III, pp. 126-156 (1961). Preferably such couplers are pyrazolones, pyrazolotriazoles, or pyrazolobenzimidazoles that form magenta dyes upon reaction with oxidized color developing agents. Especially preferred couplers are 1H-pyrazolo[5,1-c]-1,2,4-triazole and 1H-pyrazolo[1,5-b]-1,2,4-triazole. Examples of 1H-pyrazolo[5,1-c]-1,2,4-triazole couplers are described in U.K. Patent Nos. 1,247,493; 1,252,418; 1,398,979; U.S. Pat. Nos. 4,443,536; 4,514,490; 4,540,654; 4,590,153; 4,665,015; 4,822,730; 4,945,034; 5,017,465; and 5,023,170. Examples of 1H-pyrazolo[1,5-b]-1,2,4-triazoles can be found in European Patent applications 176,804; 177,765; U.S. Pat. Nos. 4,659,652; 5,066,575; and 5,250,400.

Typical pyrazoloazole and pyrazolone couplers are represented by the following formulas:



wherein R<sub>a</sub> and R<sub>b</sub> independently represent H or a substituent; R<sub>c</sub> is a substituent (preferably an aryl group); R<sub>d</sub> is a substituent (preferably an anilino, carbonamido, ureido, carbamoyl, alkoxy, aryloxycarbonyl, alkoxy carbonyl, or N-heterocyclic group); X is hydrogen or a coupling-off group; and Z<sub>a</sub>, Z<sub>b</sub>, and Z<sub>c</sub> are independently a substituted methine group, =N—, =C—, or —NH—, provided that one of either the Z<sub>a</sub>—Z<sub>b</sub> bond or the Z<sub>b</sub>—Z<sub>c</sub> bond is a double bond and the other is a single bond, and when the Z<sub>b</sub>—Z<sub>c</sub> bond is a carbon-carbon double bond, it may form part of an aromatic ring, and at least one of Z<sub>a</sub>, Z<sub>b</sub>, and Z<sub>c</sub> represents a methine group connected to the group R<sub>b</sub>.

43

Specific examples of such couplers are:



Couplers that form yellow dyes upon reaction with oxidized color developing agent are described in such representative patents and publications as: U.S. Pat. Nos. 2,298, 443; 2,407,210; 2,875,057; 3,048,194; 3,265,506; 3,447, 928; 3,960,570; 4,022,620; 4,443,536; 4,910,126; and 5,340,703 and "Farbkuppler-eine Literatur Ubersicht," published in Agfa Mitteilungen, Band III, pp. 112-126 (1961). Such couplers are typically open chain ketomethyl- 65  
ene compounds. Also preferred are yellow couplers such as described in, for example, European Patent Application Nos.

44

482,552; 510,535; 524,540; 543,367; and U.S. Pat. No. 5,238,803. For improved color reproduction, couplers which give yellow dyes that cut off sharply on the long wavelength side are particularly preferred (for example, see U.S. Pat. No. 5,360,713).

Typical preferred yellow couplers are represented by the following formulas:



45

-continued



Y-2



Y-3



Y-4



Y-5



Y-6

46

destroy properties necessary for photographic utility. When the term "group" is applied to the identification of a substituent containing a substitutable hydrogen, it is intended to encompass not only the substituent's unsubstituted form, but also its form further substituted with any group or groups as herein mentioned. Suitably, the group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolylxy; carbonamido, such as acetamido, benzamido, butyramido, tetradecanamido, alpha-(2,4-di-t-pentyl-phenoxy)acetamido, alpha-(2,4-di-t-pentylphenoxy) butyramido, alpha-(3-pentadecylphenoxy)-hexanamido, alpha-(4-hydroxy-3-t-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzyloxycarbonylamino, hexadecyloxycarbonylamino, 2,4-di-t-butylphenoxy carbonylamino, phenylcarbonylamino, 2,5-(di-t-pentylphenyl) carbonylamino, p-dodecyl-phenylcarbonylamino, p-tolylcarbonylamino, N-methylureido, N,N-dimethylureido, N-methyl-N-dodecylureido, N-hexadecylureido, N,N-dioctadecylureido, N,N-diethyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoyl, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; acyl, such as acetyl, (2,4-di-t-amyloxy)acetyl, phenoxy carbonyl, p-dodecylxyphenoxy carbonyl, methoxycarbonyl, butoxycarbonyl, tetradecyloxycarbonyl, ethoxycarbonyl, benzyloxycarbonyl, 3-pentadecyloxycarbonyl, and dodecylloxycarbonyl; sulfonyl, such as methoxysulfonyl, octyloxysulfonyl, tetradecyloxysulfonyl, 2-ethylhexyloxysulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl,

Unless otherwise specifically stated, substituent groups which may be substituted on molecules herein include any groups, whether substituted or unsubstituted, which do not

**47**

hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acetoxy, benzoyloxy, octadecanoyloxy, p-dodecylamido benzoxyloxy, N-phenylcarbamoyloxy, N-ethylcarbamoyloxy, and cyclohexylcarbonyloxy; amino, such as phenylanilino, 2-chloroanilino, diethylamino, dodecylamino; imino, such as 1 (N-phenylimido)ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

Representative substituents on ballast groups include alkyl, aryl, alkoxy, aryloxy, alkylthio, hydroxy, halogen, alkoxy carbonyl, aryloxy carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

Stabilizers and scavengers that can be used in these photographic elements, but are not limited to, the following.

ST-1



ST-2

**48**

-continued

ST-3



ST-4



ST-5



ST-6



ST-7



ST-8



ST-9



49

-continued



ST-10

50

-continued



ST-15

60



**51**

-continued



ST-24

**52**

-continued



UV-3



UV-4



UV-5

---

|                                                 |      |
|-------------------------------------------------|------|
| Tritolyl phosphate                              | S-1  |
| Dibutyl phthalate                               | S-2  |
| Diundecyl phthalate                             | S-3  |
| N,N-Diethyldodecanamide                         | S-4  |
| N,N-Dibutyldodecanamide                         | S-5  |
| Tris(2-ethylhexyl)phosphate                     | S-6  |
| Acetyl tributyl citrate                         | S-7  |
| 2,4-Di-tert-pentylphenol                        | S-8  |
| 2-(2-Butoxyethoxy)ethyl acetate                 | S-9  |
| 1,4-Cyclohexyldimethylene bis(2-ethylhexanoate) | S-10 |

---

Examples of solvents which may be used in the invention include the following:

25



UV-6

30

35

40

45

50

55

60



UV-1

45



UV-7



UV-2



UV-8

The aqueous phase may include surfactants. Surfactant may be cationic, anionic, zwitterionic or non-ionic. Useful surfactants include, but are not limited to the following:



CF<sub>3</sub>•(CF<sub>2</sub>)<sub>7</sub>•SO<sub>3</sub>Na

CH<sub>3</sub>•(CH<sub>2</sub>)<sub>n</sub>•SO<sub>3</sub>Na, n = 12-14



CH<sub>3</sub>•(CH<sub>2</sub>)<sub>11</sub>•OSO<sub>3</sub>Na



n = ca. 10



n = ca. 4



n = ca. 6, m = ca. 2



n = ca. 10



10

SF-2

SF-3

SF-4

20

Further, it is contemplated to stabilize photographic dispersions prone to particle growth through the use of hydrophobic, photographically inert compounds such as disclosed by Zengerle et al in U.S. Ser. No. 07/978,104.

In a preferred embodiment the invention employs recording elements which are constructed to contain at least three silver halide emulsion layer units. A suitable full color, multilayer format for a recording element used in the invention is represented by Structure I.

---

STRUCTURE I

---

Red-sensitized  
cyan dye image-forming silver halide emulsion unit  
Interlayer

Green-sensitized  
magenta dye image-forming silver halide emulsion unit  
Interlayer

Blue-sensitized  
yellow dye image-forming silver halide emulsion unit  
//// Support ////

---

SF-7

35

SF-8

40

45

SF-9

50

SF-10

55

SF-11

60

65

wherein the red-sensitized, cyan dye image-forming silver halide emulsion unit is situated nearest the support; next in order is the green-sensitized, magenta dye image-forming unit, followed by the uppermost blue-sensitized, yellow dye image-forming unit. The image-forming units are separated from each other by hydrophilic colloid interlayers containing an oxidized developing agent scavenger to prevent color contamination. Silver halide emulsions satisfying the grain and gelatino-peptizer requirements described above can be present in any one or combination of the emulsion layer units. Additional useful multicolor, multilayer formats for an element of the invention include structures as described in U.S. Pat. No. 5,783,373. Each of such structures in accordance with the invention preferably would contain at least three silver halide emulsions comprised of high chloride grains having at least 50 percent of their surface area bounded by {100} crystal faces and containing dopants from classes (i) and (ii), as described above. Preferably each of the emulsion layer units contains emulsion satisfying these criteria.

Conventional features that can be incorporated into multilayer (and particularly multicolor) recording elements contemplated for use in the method of the invention are illustrated by Research Disclosure, Item 38957, cited above:

XI. Layers and layer arrangements

XII. Features applicable only to color negative

XIII. Features applicable only to color positive

B. Color reversal

C. Color positives derived from color negatives

XIV. Scan facilitating features.

The recording elements comprising the radiation sensitive high chloride emulsion layers according to this invention can be conventionally optically printed, or in accordance with a particular embodiment of the invention can be

image-wise exposed in a pixel-by-pixel mode using suitable high energy radiation sources typically employed in electronic printing methods. Suitable actinic forms of energy encompass the ultraviolet, visible and infrared regions of the electromagnetic spectrum as well as electron-beam radiation and is conveniently supplied by beams from one or more light emitting diodes or lasers, including gaseous or solid state lasers. Exposures can be monochromatic, orthochromatic or panchromatic. For example, when the recording element is a multilayer multicolor element, exposure can be provided by laser or light emitting diode beams of appropriate spectral radiation, for example, infrared, red, green or blue wavelengths, to which such element is sensitive. Multicolor elements can be employed which produce cyan, magenta and yellow dyes as a function of exposure in separate portions of the electromagnetic spectrum, including at least two portions of the infrared region, as disclosed in the previously mentioned U.S. Pat. No. 4,619,892. Suitable exposures include those up to 2000 nm, preferably up to 1500 nm. Suitable light emitting diodes and commercially available laser sources are known and commercially available. Image-wise exposures at ambient, elevated or reduced temperatures and/or pressures can be employed within the useful response range of the recording element determined by conventional sensitometric techniques, as illustrated by T. H. James, *The Theory of the Photographic Process*, 4th Ed., Macmillan, 1977, Chapters 4, 6, 17, 18 and 23.

It has been observed that anionic  $[MX_xY_yL_z]$  hexacoordination complexes, where M is a group 8 or 9 metal (preferably iron, ruthenium or iridium), X is halide or pseudohalide (preferably Cl, Br or CN) x is 3 to 5, Y is  $H_2O$ , y is 0 or 1, L is a C—C, H—C or C—N—H organic ligand, and Z is 1 or 2, are surprisingly effective in reducing high intensity reciprocity failure (HIRF), low intensity reciprocity failure (LIRF) and thermal sensitivity variance and in improving latent image keeping (LIK). As herein employed HIRF is a measure of the variance of photographic properties for equal exposures, but with exposure times ranging from  $10^{-1}$  to  $10^{-6}$  second. LIRF is a measure of the variance of photographic properties for equal exposures, but with exposure times ranging from  $10^{-1}$  to 100 seconds. Although these advantages can be generally compatible with face centered cubic lattice grain structures, the most striking improvements have been observed in high (>50 mole %, preferably  $\geq 90$  mole %) chloride emulsions. Preferred C—C, H—C or C—N—H organic ligands are aromatic heterocycles of the type described in U.S. Pat. No. 5,462,849. The most effective C—C, H—C or C—N—H organic ligands are azoles and azines, either unsubstituted or containing alkyl, alkoxy or halide substituents, where the alkyl moieties contain from 1 to 8 carbon atoms. Particularly preferred azoles and azines include thiazoles, thiazolines and pyrazines.

The quantity or level of high energy actinic radiation provided to the recording medium by the exposure source is generally at least  $10^{-4}$  ergs/cm<sup>2</sup>, typically in the range of about  $10^{-4}$  ergs/cm<sup>2</sup> to  $10^{-3}$  ergs/cm<sup>2</sup> and often from  $10^{-3}$  ergs/cm<sup>2</sup> to  $10^2$  ergs/cm<sup>2</sup>. Exposure of the recording element in a pixel-by-pixel mode as known in the prior art persists for only a very short duration or time. Typical maximum exposure times are up to  $100\mu$  seconds, often up to  $10\mu$  seconds, and frequently up to only  $0.5\mu$  seconds. Single or multiple exposures of each pixel are contemplated. The pixel density is subject to wide variation, as is obvious to those skilled in the art. The higher the pixel density, the sharper the images can be, but at the expense of equipment complexity. In general, pixel densities used in conventional electronic

printing methods of the type described herein do not exceed  $10^7$  pixels/cm<sup>2</sup> and are typically in the range of about  $10^4$  to  $10^6$  pixels/cm<sup>2</sup>. An assessment of the technology of high-quality, continuous-tone, color electronic printing using silver halide photographic paper which discusses various features and components of the system, including exposure source, exposure time, exposure level and pixel density and other recording element characteristics is provided in Firth et al., *A Continuous-Tone Laser Color Printer*, Journal of Imaging Technology, Vol. 14, No. 3, June 1988, which is hereby incorporated herein by reference. As previously indicated herein, a description of some of the details of conventional electronic printing methods comprising scanning a recording element with high energy beams such as light emitting diodes or laser beams, are set forth in Hioki U.S. Pat. No. 5,126,235, European Patent Applications 479 167 A1 and 502 508 A1.

Once imagewise exposed, the recording elements can be processed in any convenient conventional manner to obtain a viewable image. Such processing is illustrated by Research Disclosure, Item 38957, cited above:

#### XVIII. Chemical development systems

#### XIX. Development

#### XX. Desilvering, washing, rinsing and stabilizing

In addition, a useful developer for the inventive material is a homogeneous, single part developing agent. The homogeneous, single-part color developing concentrate is prepared using a critical sequence of steps:

In the first step, an aqueous solution of a suitable color developing agent is prepared. This color developing agent is generally in the form of a sulfate salt. Other components of the solution can include an antioxidant for the color developing agent, a suitable number of alkali metal ions (in an at least stoichiometric proportion to the sulfate ions) provided by an alkali metal base, and a photographically inactive water-miscible or water-soluble hydroxy-containing organic solvent. This solvent is present in the final concentrate at a concentration such that the weight ratio of water to the organic solvent is from about 15:85 to about 50:50.

In this environment, especially at high alkalinity, alkali metal ions and sulfate ions form a sulfate salt that is precipitated in the presence of the hydroxy-containing organic solvent. The precipitated sulfate salt can then be readily removed using any suitable liquid/solid phase separation technique (including filtration, centrifugation or decantation). If the antioxidant is a liquid organic compound, two phases may be formed and the precipitate may be removed by discarding the aqueous phase.

The color developing concentrates of this invention include one or more color developing agents that are well known in the art that, in oxidized form, will react with dye forming color couplers in the processed materials. Such color developing agents include, but are not limited to, aminophenols, p-phenylenediamines (especially N,N-dialkyl-p-phenylenediamines) and others which are well known in the art, such as EP 0 434 097A1 (published Jun. 26, 1991) and EP 0 530 921A1 (published Mar. 10, 1993). It may be useful for the color developing agents to have one or more water-solubilizing groups as are known in the art.

Further details of such materials are provided in Research Disclosure, publication 38957, pages 592-639 (September 1996). Research Disclosure is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011). This reference will be referred to hereinafter as "Research Disclosure".

Preferred color developing agents include, but are not limited to, N,N-diethyl p-phenylenediamine sulfate (KODAK Color Developing Agent CD-2), 4-amino-3-methyl-N-(2-methane sulfonamidoethyl)aniline sulfate, 4-(N-ethyl-N-β-hydroxyethylamino)-2-methylaniline sulfate (KODAK Color Developing Agent CD-4), p-hydroxyethylaminoaniline sulfate, 4-(N-ethyl-N-2-methanesulfonylaminoethyl)-2-methylphenylenediamine sesquisulfate (KODAK Color Developing Agent CD-3), 4-(N-ethyl-N-2-methanesulfonylaminoethyl)-2-methylphenylenediamine sesquisulfate, and others readily apparent to one skilled in the art.

In order to protect the color developing agents from oxidation, one or more antioxidants are generally included in the color developing compositions. Either inorganic or organic antioxidants can be used. Many classes of useful antioxidants are known, including but not limited to, sulfites (such as sodium sulfite, potassium sulfite, sodium bisulfite and potassium metabisulfite), hydroxylamine (and derivatives thereof), hydrazines, hydrazides, amino acids, ascorbic acid (and derivatives thereof), hydroxamic acids, aminoketones, mono- and polysaccharides, mono- and polyamines, quaternary ammonium salts, nitroxy radicals, alcohols, and oximes. Also useful as antioxidants are 1,4-cyclohexadienes. Mixtures of compounds from the same or different classes of antioxidants can also be used if desired.

Especially useful antioxidants are hydroxylamine derivatives as described for example, in U.S. Pat. No. 4,892,804, U.S. Pat. No. 4,876,174, U.S. Pat. No. 5,354,646, and U.S. Pat. No. 5,660,974, all noted above, and U.S. Pat. No. 5,646,327 (Burns et al). Many of these antioxidants are mono- and dialkylhydroxylamines having one or more substituents on one or both alkyl groups. Particularly useful alkyl substituents include sulfo, carboxy, amino, sulfonamido, carbonamido, hydroxy and other solubilizing substituents.

More preferably, the noted hydroxylamine derivatives can be mono- or dialkylhydroxylamines having one or more hydroxy substituents on the one or more alkyl groups. Representative compounds of this type are described for example in U.S. Pat. No. 5,709,982 (Marrese et al) as having the structure:



wherein R is hydrogen, a substituted or unsubstituted alkyl group of 1 to 10 carbon atoms, a substituted or unsubstituted hydroxyalkyl group of 1 to 10 carbon atoms, a substituted or unsubstituted cycloalkyl group of 5 to 10 carbon atoms, or a substituted or unsubstituted aryl group having 6 to 10 carbon atoms in the aromatic nucleus.

X<sub>1</sub> is —CR<sub>2</sub>(OH)CHR<sub>1</sub>— and X<sub>2</sub> is —CHR<sub>1</sub>CR<sub>2</sub>(OH)— wherein R<sub>1</sub> and R<sub>2</sub> are independently hydrogen, hydroxy, a substituted or unsubstituted alkyl group of 1 or 2 carbon atoms, a substituted or unsubstituted hydroxyalkyl group of 1 or 2 carbon atoms, or R<sub>1</sub> and R<sub>2</sub> together represent the carbon atoms necessary to complete a substituted or unsubstituted 5- to 8-membered saturated or unsaturated carbocyclic ring structure.

Y is a substituted or unsubstituted alkylene group having at least 4 carbon atoms, and has an even number of carbon atoms, or Y is a substituted or unsubstituted divalent aliphatic group having an even total number of carbon and oxygen atoms in the chain, provided that the aliphatic group has a least 4 atoms in the chain.

Also in Structure I, m, n and p are independently 0 or 1. Preferably, each of m and n is 1, and p is 0.

Specific di-substituted hydroxylamine antioxidants include, but are not limited to: N,N-bis(2,3-dihydroxypropyl)hydroxylamine, N,N-bis(2-methyl-2,3-dihydroxypropyl)hydroxylamine and N,N-bis(1-hydroxymethyl-2-hydroxy-3-phenylpropyl)hydroxylamine. The first compound is preferred.

The following examples illustrate the practice of this invention. They are not intended to be exhaustive of all possible variations of the invention. Parts and percentages are by weight unless otherwise indicated.

## EXAMPLES

### Example 1

In this example two iterations of the invention (sample 1 and 2) are compared to a typical polyethylene melt cast imaging support (sample 4) and a imaging support consisting of biaxially oriented polyolefin sheets laminated to paper (sample 3). This example will show that the invention support materials are superior to prior art imaging support materials for tear resistance. Further, it will be obvious that the invention materials are also superior for image whiteness and opacity.

Photographic grade cellulose paper used in the example:

A photographic paper support was produced by refining a pulp furnish of 50% bleached hardwood kraft, 25% bleached hardwood sulfite, and 25% bleached softwood sulfite through a double disk refiner, then a Jordan conical refiner to a Canadian Standard Freeness of 200 cc. To the resulting pulp furnish was added 0.2% alkyl ketene dimer, 1.0% cationic cornstarch, 0.5% polyamide-epichlorohydrin, 0.26 anionic polyacrylamide, and 5.0% TiO<sub>2</sub> on a dry weight basis. An about 147 g/m<sup>2</sup> bone dry weight base paper was made on a fourdrinier paper machine, wet pressed to a solid of 42%, and dried to a moisture of 10% using steam-heated dryers achieving a Sheffield Porosity of 160 Sheffield Units and an apparent density 0.70 g/cc. The paper base was then surface sized using a vertical size press with a 10% hydroxyethylated cornstarch solution to achieve a loading of 3.3 wt. % starch. The surface sized support was calendered to an apparent density of 1.04 gm/cc.

Sample 1 (invention):

Layers 2 to 4 were prepared by cast extruding as an integral sheet on a chill roll, drafted in the machine direction and then in the transverse direction (approximately 3x3). A layer (L3) of microvoided polyester (polyethylene terephthalate) comprising polyester and microbeads with a layer thickness of 25  $\mu\text{m}$  and a percent voiding of 50%. The voiding agent was a cross-linked microbead of polystyrene with divinylbenzene in the amount of 50% by weight of said layer. The mean particle size of the microbead was between 1 to 2  $\mu\text{m}$  and were coated with a slip agent of colloidal alumina. The top, middle, and bottom layers were coextruded through a standard three slot coat hanger die at 265° C. onto a chill roll controlled at a temperature between 50–60° C. The three layer film was stretched biaxially using a standard laboratory film stretching unit at a temperature of 105° C.

The preparation steps for the cross-linked microbeads used to void the middle layer of the coextruded support were as follows:

(1) The microbeads were prepared by conventional aqueous suspension polymerization to give nearly monodisperse bead diameters from 2 to 20  $\mu\text{m}$  and at levels of cross-linking from 5 mol % to 30 mol %.

(2) After separation and drying, the microbeads were compounded on conventional twin-screw extrusion equipment into the polyester at level of 25% by weight and pelletized to form a concentrate, suitable for let-down to lower loadings.

(3) The microbead concentrate pellets were mixed with virgin pellets and dried using standard conditions for polyethylene terephthalate, 170–180° C. convection with desiccated air for between 4–6 hours.

The L1 gel sub/primer is applied to the cast sheet by coating a thin layer of primer and then coating a thin gelatin layer on the primer. The sheet was then laminated to the paper base with a melt extruded blend of polyethylene and anhydride-modified ethylene acrylate at 365° C. The polyester sheet, melt polymer and paper were simultaneously brought together into the chilled pressure nip. The L8 layer is a commercially available biaxially oriented sheet of polypropylene and was attached to the paper base with a melt polymer being extruded into a pressure nip. The writable/conductive layer is applied by a roller coating method on the cornea treated surface of the terpolymer skin

The support structure for sample 1 is listed below:

L1: Aqueous gelatin sub coating

L2: Polyester with 24% anatase TiO<sub>2</sub> and optical brightener at 8 micrometer

L3: Voided polyester 25 micrometers thick with a density of 0.84 g/cc

L4: Polyester with 18% rutile TiO<sub>2</sub> at 8 micrometers thick

L5: Bonding layer consisting a 20%/80% blend of Dupont Bynel and a extrusion grade low density polyethylene melt extruded at 12 g/m<sup>2</sup>

L6: Imaging grade cellulose base paper

L7: Bonding layer consisting a 20%/80% blend of Dupont Bynel and a extrusion grade low density polyethylene melt extruded at 12 g/m<sup>2</sup>

L8: Polyester with a skin of a copolymer of polyethylene and a terpolymer of ethylene propylene and butylene

L9: Styrene butadiene methacrylate coating

Sample 2 (invention):

Layers 1 to 5 may be prepared by cast extruding as an integral sheet on a chill roll, drafted in the machine direction and then in the transverse direction (approximately 3×3). A layer (L3) of mircovoiced polyester (polyethylene terephthalate) comprising polyester and microbeads with a layer thickness of 25 μm and a percent voiding of 50%. The voiding agent was a cross-linked microbead of polystyrene with divinylbenzene in the amount of 50% by weight of said layer. The mean particle size of the microbead was between 1 to 2 μm and were coated with a slip agent of colloidal alumina. The layers were coextruded through a standard three slot coat hanger die at 265° C. onto a chill roll controlled at a temperature between 50–60° C. The five layer film was stretched biaxially using a standard laboratory film stretching unit at a temperature of 105° C.

The preparation steps for the cross-linked microbeads used to void the middle layer of the coextruded support were as follows:

(1) The microbeads were prepared by conventional aqueous suspension polymerization to give nearly mono-disperse bead diameters from 2 to 20 μm and at levels of cross-linking from 5 mol % to 30 mol %.

(2) After separation and drying, the microbeads were compounded on conventional twin-screw extrusion equipment into the polyester at level of 25% by weight and pelletized to form a concentrate, suitable for let-down to lower loadings.

(3) The microbead concentrate pellets were mixed with virgin pellets and dried using standard conditions for polyethylene terephthalate, 170–180° C. convection with desiccated air for between 4–6 hours.

5 The bottom layer of the coextruded support was a solid layer of polyester with an intrinsic viscosity of at about 0.68 cp.

A layer (L2) of polyester with a layer thickness of 8.0 μm. The polyester layer contained 0.12% by weight of optical brightener, 24% by weight of TiO<sub>2</sub>. The optical brightener used was Hostalux KS manufactured by Ciba-Geigy. The rutile TiO<sub>2</sub> used was DuPont R104 (a 0.22 micrometer particle size TiO<sub>2</sub>).

10 A layer of low density polyethylene with a layer thickness of 0.75 μm. The polyethylene layer blue tint (Pigment Blue 60).

The sheet was then laminated to the paper base with a melt extruded blend of polyethylene and anhydride-modified ethylene acrylate at 365° C. The polyester sheet, melt polymer and paper were simultaneously brought together into the chilled pressure nip. The L9 layer is a commercially available biaxially oriented sheet of polypropylene and was attached to the paper base with a melt polymer being extruded into a pressure nip. The writable/conductive layer is applied by a roller coating method on the cornea treated surface of the terpolymer surface.

15 The imaging support structure for sample 2 is listed below:

L1: 0.75 μm low density polyethylene with red and blue pigments

L2: Polyester with 24% anatase TiO<sub>2</sub> and optical brightener at 8 μm

L3: Voided polyester 25 μm thick with a density of 0.89 g/cc

L4: Polyester with 24% anatase TiO<sub>2</sub> at 8 μm thick

L5: Bonding layer consisting a 20%/80% blend of DuPont Bynel and an extrusion grade low density polyethylene melt extruded at 12 g/m<sup>2</sup>

L6: Imaging grade cellulose base paper

L7: Bonding layer consisting a 20%/80% blend of DuPont Bynel and an extrusion grade low density polyethylene melt extruded at 12 g/m<sup>2</sup>

L8: Polyester with a skin of a copolymer of polyethylene and a terpolymer of ethylene propylene and butylene

L9: Styrene butadiene methacrylate coating

#### Example 3 (control)

50 Commercially available Eastman Kodak Ektatherm XLS Thermal dye transfer reflective receiver. This imaging support materials has a paper base laminated on the top and bottom sides with biaxially oriented polyolefin sheets.

#### Example 4 (control)

Typical color photographic paper consisting of a two side polyethylene melt cast coating on a photographic grade paper base.

60 Tear resistance for the imaging supports elements is the amount of force required to start a tear along an edge of the photographic element. The tear resistance test used was originally proposed by G. G. Gray and K. G. Dash, Tappi Journal 57, pages 167–170 published 1974. The tear resistance for the photographic elements is determined by the tensile strength and the stretch of the photographic element. A 15 mm×25 mm sample is looped around a metal cylinder

with a 2.5 cm diameter. The two ends of the sample are clamped by a Instron tensile tester. A load is applied to the sample at a rate of 2.5 cm per minute until a tear is observed at which time the load expressed in N, is recorded. The tear resistance was measured for the four samples (samples 1-4) of this example. The tear resistance mean values are listed in Table 1 below:

TABLE 1

| Sample        | Tear Resistance (N) |
|---------------|---------------------|
| 1 (invention) | 1124                |
| 2 (invention) | 1078                |
| 3 (control)   | 675                 |
| 4 (control)   | 135                 |

The results above clearly demonstrate that the use of a polyester biaxially oriented sheets laminated to paper are higher in tear resistance than biaxially oriented polyolefin sheets laminated to cellulose paper and significant higher in tear resistance than typical polyethylene cast coated photographic support materials. Tear resistant support materials are perceptually preferred in that they offer the consumer image durability as images are viewed, displayed and stored. The improvement in tear resistance of imaging support materials of the invention also improves the web transport efficiency and picking efficiency of digital printing equipment such as an ink jet printers or a thermal dye transfer printers. Finally, the increased amount of  $TiO_2$  utilized in the invention support material would result in a brighter, whiter, sharper image with improved image opacity.

The invention has been described in detail with particular reference to certain preferred embodiments thereof, but it will be understood that variations and modifications can be effected within the spirit and scope of the invention.

What is claimed is:

- An imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer at least one upper solid polymer layer and below said voided polyester layer at least one lower solid polymer layer, and at least one backside oriented polymer sheet below said base paper, and wherein at least one upper polymer layer comprises a white pigment wherein at least one upper solid polymer layer comprises polyethylene.
- The imaging element of claim 1 wherein said at least one upper solid polymer layer comprising polyethylene forms the upper surface of the upper biaxially oriented sheet.
- The imaging element of claim 1 wherein the upper solid polyethylene polymer layer comprises tinting agents.
- The imaging element of claim 1 wherein said upper solid polymer layer comprises optical brighteners and white pigment.
- The imaging element of claim 1 wherein at least one layer of said integrally formed biaxially oriented sheet comprises fluoropolymers.
- The imaging element of claim 1 wherein said integrally formed biaxially oriented polymer sheet has a modulus of at least 690 MPa.
- The imaging element of claim 6 wherein said integral layer is adhered to said base paper utilizing a layer of an anhydride-modified ethylene acrylate.
- The imaging element of claim 6 wherein said integrally formed biaxially oriented sheet has a Young's modulus of between 690 and 15,000 MPa.
- The imaging element of claim 1 wherein at least one voided layer has a void volume of between 2 and 60 percent.
- The imaging element of claim 1 wherein said integrally formed biaxially oriented sheet comprises titanium dioxide in an amount between 12 and 60 percent by weight.
- The imaging element of claim 1 wherein said integrally formed biaxially oriented sheets has a water vapor transmission rate of less than 20 g/m<sup>2</sup>/day.
- The imaging element of claim 1 wherein said integrally formed biaxially oriented sheet further comprises hindered amine light stabilizers.
- The imaging element of claim 1 wherein said at least one backside oriented sheet comprises polyester polymer.
- The imaging element of claim 1 wherein said at least one backside oriented sheet is provided with indicia on its upper surface.
- The imaging element of claim 1 wherein said at least one backside oriented sheet is provided with a magnetic layer.
- The imaging element of claim 1 wherein said at least one backside oriented sheet has a bottom surface roughness of between 0.2 and 2.0  $\mu$ m.
- The imaging element of claim 1 wherein said at least one backside oriented sheet is a biaxially oriented sheet.
- The imaging element of claim 1 wherein said at least one backside oriented sheet comprises a rough lower surface polymer layer and a layer having a modulus of greater than 690 MPa.
- The imaging element of claim 1 wherein said base paper comprises a cellulose fiber paper having a Young's modulus in the machine direction of between 2,700 and 15,000 MPa and a Young's modulus in the machine cross direction of between 1,200 and 8,000 MPa.
- The imaging element of claim 1 further comprising at least one photosensitive silver halide layer.
- The imaging element of claim 1 further comprising at least one ink jet receiving layer.
- The imaging element of claim 1 further comprising at least one imaging layer.
- An imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer at least one upper solid polymer layer and below said voided polyester layer at least one lower solid polymer layer, and at least one backside oriented polymer sheet below said base paper, and wherein at least one upper polymer layer comprises a white pigment and wherein at least one layer of said integrally formed biaxially oriented sheet comprises fluoropolymers.
- The imaging element of claim 24 wherein at least one upper solid polymer layer comprises tinting agents.
- The imaging element of claim 25 wherein at least one upper solid polymer layer comprises polyethylene.
- The imaging element of claim 24 wherein at least one upper solid polymer layer comprises optical brighteners.
- The imaging element of claim 24 wherein said integrally formed biaxially oriented polymer sheet has a modulus of at least 690 MPa.
- The imaging element of claim 28 wherein said integral layer is adhered to said base paper utilizing a layer of an anhydride-modified ethylene acrylate.
- The imaging element of claim 28 wherein said integrally formed biaxially oriented sheet has a Young's modulus of between 690 and 15,000 MPa.

63

**31.** The imaging element of claim **24** wherein said integrally formed biaxially oriented sheet comprises titanium dioxide in an amount between 12 and 60 percent by weight.

**32.** The imaging element of claim **24** wherein said integrally formed biaxially oriented sheets has a water vapor transmission rate of less than 20 g/m<sup>2</sup>/day.

**33.** The imaging element of claim **26** wherein said integrally formed biaxially oriented sheet further comprises hindered amine light stabilizers.

**34.** The imaging element of claim **24** wherein said at least one backside oriented sheet comprises polyester polymer.

**35.** The imaging element of claim **24** wherein said base paper comprises a cellulose fiber paper having a Young's modulus in the machine direction of between 2,700 and 15,000 MPa and a Young's modulus in the machine cross direction of between 1,200 and 8,000 MPa.

**36.** The imaging element of claim **24** further comprising at least one photosensitive silver halide layer.

**37.** The imaging element of claim **24** further comprising at least one ink jet receiving layer.

**38.** The imaging element of claim **24** further comprising at least one imaging layer.

**39.** An imaging element comprising a base paper having adhered to its upper surface an integrally formed biaxially oriented polymer sheet comprising at least three layers, wherein said integrally formed biaxially oriented polymer sheet comprises at least one layer of voided polyester polymer and above said voided polyester layer at least one upper solid polymer layer and below said voided polyester layer at least one lower solid polymer layer, and at least one

64

backside oriented polymer sheet below said base paper, and wherein at least one upper polymer layer comprises a white pigment wherein said integrally formed biaxially oriented sheet further comprises hindered amine light stabilizers.

**40.** The imaging element of claim **39** wherein at least one upper solid polymer layer comprises optical brighteners.

**41.** The imaging element of claim **40** wherein at least one upper solid polymer layer comprises polyethylene.

**42.** The imaging element of claim **40** wherein at least one upper solid polymer layer comprises tinting agents.

**43.** The imaging element of claim **39** wherein said integrally formed biaxially oriented sheet comprises titanium dioxide in an amount between 12 and 60 percent by weight.

**44.** The imaging element of claim **39** wherein said at least one backside oriented sheet comprises polyester polymer.

**45.** The imaging element of claim **39** wherein said at least one backside oriented sheet is provided with indicia on its upper surface.

**46.** The imaging element of claim **39** further comprising at least one photosensitive silver halide layer.

**47.** The imaging element of claim **39** further comprising at least one ink jet receiving layer.

**48.** The imaging element of claim **39** further comprising at least one imaging layer.

**49.** The imaging element of claim **39** wherein said integrally formed biaxially oriented polymer sheet has a modulus of at least 690 MPa.

\* \* \* \* \*